



US008475984B1

(12) **United States Patent**  
**Hirose et al.**

(10) **Patent No.:** **US 8,475,984 B1**  
(b4) **Date of Patent:** **Jul. 2, 2013**

(54) **IMAGE HOLDING MEMBER FOR IMAGE FORMING APPARATUS, PROCESS CARTRIDGE, AND IMAGE FORMING APPARATUS**

(75) Inventors: **Hidekazu Hirose**, Kanagawa (JP); **Ryosaku Igarashi**, Kanagawa (JP); **Katsuhiro Sato**, Kanagawa (JP)

(73) Assignee: **Fuji Xerox Co., Ltd.**, Tokyo (JP)

(\*) Notice: Subject to any disclaimer, the term of this patent is extended or adjusted under 35 U.S.C. 154(b) by 0 days.

(21) Appl. No.: **13/466,634**

(22) Filed: **May 8, 2012**

(30) **Foreign Application Priority Data**

Dec. 22, 2011 (JP) ..... 2011-282341

(51) **Int. Cl.**

**G03G 5/06** (2006.01)  
**G03G 5/07** (2006.01)

(52) **U.S. Cl.**

CPC ..... **G03G 5/0629** (2013.01); **G03G 5/076** (2013.01)

USPC ..... **430/75**; 430/58.15; 430/59.6

(58) **Field of Classification Search**

CPC ..... G03G 5/0629; G03G 5/076

USPC ..... 430/76, 59.6, 58.15; 399/159

See application file for complete search history.

(56) **References Cited**

U.S. PATENT DOCUMENTS

4,047,948 A 9/1977 Horgan  
4,299,897 A 11/1981 Stolka et al.  
5,049,464 A \* 9/1991 Kanemaru et al. ..... 430/58.15

FOREIGN PATENT DOCUMENTS

JP A-61-132955 6/1986  
JP A-62-267749 11/1987

(Continued)

OTHER PUBLICATIONS

English language machine translation of JP 2009-064882 (Mar. 2009).\*

(Continued)

*Primary Examiner* — Christopher Rodee

(74) *Attorney, Agent, or Firm* — Oliff & Berridge, PLC

(57) **ABSTRACT**

An image holding member for an image forming apparatus includes a support and a photosensitive layer disposed on the support and containing a compound represented by following formula (I), wherein R<sup>1</sup>'s each independently represent a substituted or unsubstituted linear or branched alkyl group having from 1 to 8 carbon atoms; Ar's each independently represent a substituted or unsubstituted phenyl group, a substituted or unsubstituted monovalent polynuclear aromatic hydrocarbon group having two aromatic rings, a substituted or unsubstituted monovalent condensed aromatic hydrocarbon group having two or three aromatic rings, or a substituted or unsubstituted monovalent aromatic heterocyclic group; and n's each independently represent a number of from 0 to 7.

(I)



**6 Claims, 5 Drawing Sheets**

1



FOREIGN PATENT DOCUMENTS

|    |              |           |
|----|--------------|-----------|
| JP | A-3-138654   | 6/1991    |
| JP | 05105676 A   | * 4/1993  |
| JP | 07287408 A   | * 10/1995 |
| JP | 2009064882 A | * 3/2009  |

OTHER PUBLICATIONS

English language machine translation of JP 05-105676 (Apr. 1993).\*  
English language machine translation of JP 07-287408 (Oct. 1995).\*

\* cited by examiner

FIG. 1



FIG. 2



FIG. 3



FIG. 4



FIG. 5



**IMAGE HOLDING MEMBER FOR IMAGE FORMING APPARATUS, PROCESS CARTRIDGE, AND IMAGE FORMING APPARATUS**

**CROSS-REFERENCE TO RELATED APPLICATIONS**

This application is based on and claims priority under 35 USC 119 from Japanese Patent Application No. 2011-282341 filed Dec. 22, 2011.

**BACKGROUND**

1. Technical Field

The present invention relates to an image holding member for an image forming apparatus, a process cartridge, and an image forming apparatus.

2. Related Art

A photoreceptor having a photosensitive layer which contains an organic photoconductive compound as a principal component has many advantages such as relatively easy manufacturability, low price, easy handleability, and excellent thermal stability, as compared with photoreceptors containing conventionally used inorganic photoconductors (selenium, zinc oxide, cadmium sulfide, silicon and the like) as principal components. Thus, active investigations have been conducted thereon.

Particularly, photoreceptors having a functionally separable, laminate type photosensitive layer, in which the charge generation function, and the charge transport function of the photoconductor are respectively assigned to separate functional layers, and a material having the former generation function is incorporated into a charge generating layer, while a material having the latter transport function is incorporated into a charge transport layer, have already been put to practical use.

**SUMMARY**

According to an aspect of the present invention, there is provided an image holding member for an image forming apparatus, the member having a support, and a photosensitive layer disposed on the support and containing a compound represented by the following formula (I):



wherein in the formula (I), R¹'s each independently represent a substituted or unsubstituted linear or branched alkyl group having from 1 to 8 carbon atoms; Ar's each independently represent a substituted or unsubstituted phenyl group, a substituted or unsubstituted monovalent polynuclear aromatic hydrocarbon group having two aromatic rings, a substituted

or unsubstituted monovalent condensed aromatic hydrocarbon group having two or three aromatic rings, or a substituted or unsubstituted monovalent aromatic heterocyclic group; and n's each independently represent a number of from 0 to 7.

**BRIEF DESCRIPTION OF THE DRAWINGS**

Exemplary embodiments of the present invention will be described in detail based on the following figures, wherein:

FIG. 1 is a schematic cross-sectional view of the image holding member for an image forming apparatus related to the first exemplary embodiment;

FIG. 2 is a schematic cross-sectional view of the image holding member for an image forming apparatus related to the second exemplary embodiment;

FIG. 3 is a schematic cross-sectional view of the image holding member for an image forming apparatus related to the third exemplary embodiment;

FIG. 4 is a schematic configuration diagram of an image forming apparatus related to the exemplary embodiments; and

FIG. 5 is a schematic configuration diagram of a process cartridge related to the exemplary embodiments.

**DETAILED DESCRIPTION**

Hereinafter, exemplary embodiments of the present invention will be described.

In the exemplary embodiment of the present invention, there is provided an image holding member for an image forming apparatus, which uses at least one of a compound represented by the following formula (I) and a compound represented by the following formula (II-1) as a charge transporting material. That is, the image holding member is an image holding member for an image forming apparatus, in which a photosensitive layer is formed on a support (for example, a conductive support), and the photosensitive layer contains at least one of a compound represented by the following formula (I) and a compound represented by the following formula (II-1).

Meanwhile, the conductive support according to the exemplary embodiment refers to a support having a volume resistivity of the surface of less than  $10^7 \Omega\cdot\text{cm}$  as measured based on JIS K 7194 "Testing method for resistivity of conductive

plastics with a four-point probe array". That is, the conductive support may be a support formed of a conductive material having a volume resistivity measured based on the above-described method of less than  $10^7 \Omega\cdot\text{cm}$ , or may be a support having a conductive layer formed of the conductive material on the base material surface.

The photosensitive layer in the image holding member for an image forming apparatus may be any of a single-layer type photosensitive layer containing a charge generating material and a charge transporting material in the same layer, and a functionally separated photosensitive layer in which a layer containing a charge generating material and a layer containing a charge transporting material are provided separately but adjacently to each other. As the charge transporting material, at least one of a compound represented by the following formula (I) and a compound represented by the following formula (II-1) is incorporated.

Furthermore, as the charge generating material, any known charge generating material such as oxytitanium phthalocyanine, chlorogallium phthalocyanine or hydroxygallium phthalocyanine may be used. Meanwhile, the image holding member for an image forming apparatus may include a protective layer on the outermost surface (farthest position from the conductive support), and the protective layer in this case preferably contains a crosslinkable silicone resin having charge transporting properties.

(Image Holding Member for Image Forming Apparatus)

The image holding member for an image forming apparatus related to the exemplary embodiment is an image holding member for an image forming apparatus in which a photosensitive layer containing at least one of a compound represented by the following formula (I) and a compound represented by the following formula (II-1) is formed on a support.

<Compound Represented by Formula (I)>

Hereinafter, the compound represented by the following formula (I) will be described in detail.

In the formula (I), when the alkyl group represented by R<sup>1</sup> has a substituent, the substituent may be an aryl group or a heterocyclic group.

The aryl group as the substituent preferably has from 6 to 20 carbon atoms, and examples thereof include a phenyl group, a toluoyl group, and a naphthyl group.

The heterocyclic group as the substituent means a group having a ring containing elements other than carbon and hydrogen (that is, a heterocyclic ring). The heterocyclic ring is preferably such that the number of atoms constituting the ring skeleton (Nr) is 5 or 6. The type and number of the atoms other than carbon atoms constituting the ring skeleton (heteroatoms) are not particularly limited, but for example, sulfur atoms, nitrogen atoms, oxygen atoms, selenium atoms, silicon atoms, and phosphorus atoms are preferably used. The ring skeleton may contain two or more kinds of heteroatoms, or may also contain two or more heteroatoms.

As a 5-membered heterocyclic ring, for example, thiophene, pyrrole, furan, imidazole, oxazole, selenophene, thiazole, thiadiazole, pyrazole, isoxazole, isothiazole, silole, or a heterocyclic ring in which the carbon atoms at the 3-position and the 4-position of one of the above-described compounds have been replaced by nitrogen atoms, is preferably used. Other examples of an aromatic heterocyclic ring having a 5-membered heterocyclic ring include benzothiophene, benzimidazole, and indole.

As a 6-membered heterocyclic ring, pyridine, pyrimidine, pyrazine or piperazine is preferably used.

Meanwhile, the heterocyclic group as the substituent encompasses a group in which the heterocyclic ring is sub-



In the formula (I), R<sup>1</sup>'s each independently represent a substituted or unsubstituted, linear or branched alkyl group having from 1 to 8 carbon atoms; Ar's each independently represent a substituted or unsubstituted phenyl group, a substituted or unsubstituted monovalent polynuclear aromatic hydrocarbon group having two aromatic rings, a substituted or unsubstituted monovalent condensed aromatic hydrocarbon group having two or three aromatic rings, or a substituted or unsubstituted monovalent aromatic heterocyclic group; and n's each independently represent a number of from 0 to 7.

R<sup>1</sup> in the formula (I) will be explained.

As described above, R<sup>1</sup>'s in the formula (I) each independently represent a substituted or unsubstituted, linear or branched alkyl group having from 1 to 8 carbon atoms.

The alkyl groups represented by R<sup>1</sup>'s each independently have preferably from 1 to 6 carbon atoms, and more preferably from 1 to 4 carbon atoms.

The alkyl group represented by R<sup>1</sup> is linear or branched, and from the viewpoints of maintaining crystallinity and solubility, the alkyl group is preferably a linear alkyl group.

stituted with an aromatic ring, and also encompasses a group in which an aromatic ring is substituted with a heterocyclic ring.

Specific examples of the alkyl group represented by R<sup>1</sup> in the formula (I) include a methyl group, an ethyl group, a propyl group, an n-butyl group, a t-butyl group, an n-hexyl group, and an n-octyl group. The alkyl group is preferably a methyl group, an ethyl group, a propyl group, an n-butyl group, a t-butyl group, an n-hexyl group or an n-octyl group, and more preferably a methyl group or a butyl group. When the alkyl group is a methyl group or a butyl group, it is more desirable from the viewpoints of the ease of production and the maintenance of crystallinity, and a methyl group is even more desirable from the viewpoint of easy availability.

Furthermore, R<sup>1</sup> is a substituted or unsubstituted, linear or branched alkyl group having from 1 to 8 carbon atoms, and within this range, the influence of the difference in the type of the alkyl group on the ionization potential or charge trans- portability is small.

Furthermore, the plural R<sup>1</sup>'s in the formula (I) may be identical with or different from each other, but from the viewpoint of production, it is preferable that R<sup>1</sup>'s be identical.

Ar in the formula (I) will be described

In the formula (I), Ar's each independently represent a substituted or unsubstituted phenyl group, a substituted or unsubstituted monovalent polynuclear aromatic hydrocarbon group having two aromatic rings, a substituted or unsubstituted monovalent condensed aromatic hydrocarbon group having two or three aromatic rings, or a substituted or unsubstituted monovalent aromatic heterocyclic group.

Meanwhile, the two Ar's present in the formula (I) may be identical with or different from each other, but production is easier when Ar's are identical.

Here, the polynuclear aromatic hydrocarbon group and the condensed aromatic hydrocarbon group according to the exemplary embodiment specifically mean groups having polycyclic aromatic rings that are defined below (that is, polynuclear aromatic hydrocarbon or condensed aromatic hydrocarbon).

That is, the "polynuclear aromatic hydrocarbon" represents a hydrocarbon in which two or more aromatic rings composed of carbon and hydrogen are present, and the rings are bonded by a carbon-carbon bond. A specific example is biphenyl. Furthermore, the "condensed aromatic hydrocarbon" represents a hydrocarbon compound in which two or more aromatic rings composed of carbon and hydrogen are present, and these aromatic rings share a pair of carbon atoms that are adjacently bonded to each other. Specific examples include naphthalene, anthracene, phenanthrene, and fluorene.

Furthermore, in the formula (I), the aromatic heterocyclic group selected as a structure representing Ar according to the exemplary embodiment means a group having an aromatic heterocyclic ring such as defined below.

That is, the "aromatic heterocyclic ring" represents an aromatic ring containing elements in addition to carbon and hydrogen, and for example, at least any aromatic heterocyclic ring in which the number of atoms constituting the ring skeleton (Nr) is 5 or 6 may be used. Furthermore, the type and number of the atoms that constitute the ring skeleton other than carbon atoms (heteroatoms) are not particularly limited, but for example, sulfur atoms, nitrogen atoms, and oxygen atoms are used. In the ring skeleton, at least any of two or more kinds of heteroatoms, and two or more heteroatoms may be included. Particularly, as a heterocyclic ring having a 5-membered ring structure, for example, thiophene, pyrrole, furan, or a heterocyclic ring in which the carbon atoms at the 3-position and the 4-position of any one of the above-described compounds have been replaced by nitrogen atoms is used. As a heterocyclic ring having a 6-membered ring structure, for example, pyridine is used.

Also, it is sufficient that the aromatic heterocyclic ring has the aromatic heterocyclic ring described above, and examples thereof may also include, in addition to a group composed of the aromatic heterocyclic ring described above, any of a group in which an aromatic ring is substituted with the aromatic heterocyclic ring, and a group in which the aromatic heterocyclic ring is substituted with an aromatic ring. Specific examples of the aromatic ring include the aromatic rings described above.

That is, the aromatic heterocyclic group may be, for example, a group in which one or more aromatic rings in the polycyclic aromatic ring described above (that is, the monovalent polynuclear aromatic hydrocarbon having two or more aromatic rings, or the monovalent condensed aromatic hydrocarbon having two or more aromatic rings) have been replaced by an aromatic heterocyclic ring(s), and specific examples include a thiophenylphenyl group, a phenylpyridine group, and a phenylpyrrole group.

In the formula (I), examples of the substituent which further substitutes the phenyl group, polynuclear aromatic hydrocarbon group, condensed aromatic hydrocarbon group or aromatic heterocyclic group represented by Ar, include a hydrogen atom, an alkyl group, an alkoxy group, an aryl group, an aralkyl group, a substituted amino group, and a halogen atom.

The alkyl group may be, for example, an alkyl group having from 1 to 10 carbon atoms, and examples thereof include 10 a methyl group, an ethyl group, a propyl group, and an isopropyl group.

The alkoxy group may be, for example, an alkoxy group having from 1 to 10 carbon atoms, and examples thereof include a methoxy group, an ethoxy group, a propoxy group 15 and an isopropoxy group.

The aryl group may be, for example, an aryl group having from 6 to 20 carbon atoms, and examples thereof include a phenyl group, and a toluoyl group.

The aralkyl group may be, for example, an aralkyl group 20 having from 7 to 20 carbon atoms, and examples thereof include a benzyl group and a phenethyl group.

Examples of the substituent for the substituted amino group include an alkyl group, an aryl group, and an aralkyl group, and specific examples thereof are as described above.

25 Among others, Ar in the formula (I) is preferably a substituted or unsubstituted phenyl group or a substituted or unsubstituted polynuclear aromatic hydrocarbon group from the viewpoints of mobility and easy handleability, more preferably a substituted or unsubstituted phenyl group or a substituted or unsubstituted polynuclear aromatic hydrocarbon group which does not contain a condensed aromatic hydrocarbon group and an aromatic heterocyclic ring, and even more preferably a substituted or unsubstituted phenyl group or a substituted or unsubstituted polynuclear aromatic hydrocarbon group in which the carbon atoms constituting the aromatic ring are directly bonded by a carbon-carbon bond.

Furthermore, the number of aromatic rings for Ar in the formula (I) is preferably from 1 to 6, more preferably from 1 to 3, and even more preferably 1 or 2, from the viewpoints of 40 compatibility with resins and ease of synthesis. That is, Ar in the formula (I) is more preferably a substituted or unsubstituted phenyl group, a substituted or unsubstituted biphenyl group, or a substituted or unsubstituted terphenyl group, and even more preferably an unsubstituted phenyl group, an unsubstituted biphenyl group, or an unsubstituted terphenyl group.

n in the formula (I) will be described.

n's in the formula (I) are each independently a number of 45 from 0 to 7. Two n's in the formula (I) may be identical with or different from each other, but from the viewpoint of manufacturability, it is preferable that n's be identical. It is preferable that n in the formula (I) be smaller from the viewpoint of charge transportability; however, if n is too small, the charge mobility is decreased due to the influence of the dipole moment of the carbonyl group. Therefore, n is preferably from 1 to 3, and most preferably 1.

Since the compound represented by the formula (I) has a dibenzothiophene skeleton, it can be contemplated that the compound has satisfactory charge transportability and also 50 satisfactory compatibility with resins.

<Method for Producing Compound Represented by Formula (I)>

Hereinafter, the method for producing the compound represented by the formula (I) will be specifically described.

65 As the method for synthesizing the compound having a dibenzothiophene skeleton of the exemplary embodiment, for example, a method of utilizing cross coupling biaryl synthesis

may be used. Specific examples of the cross-coupling biaryl synthesis include the Suzuki reaction, the Kharasch reaction, the Negishi reaction, the Stille reaction, the Grignard reaction, and the Ullmann reaction.

For example, synthesis may be carried out as described below, but the method is not limited to this.

(NHMe<sub>2</sub>), trimethylamine (NMe<sub>3</sub>), 1,8-diazabicyclo[5.4.0]-7-undecene (DBU), N,N-dimethyl-4-aminopyridine (DMAP), or pyridine is used.

The solvent may be any solvent which does not markedly impede the reaction, and for example, an aromatic hydrocarbon solvent such as benzene, toluene, xylene or mesitylene;



In the formula (III) and formula (IV), X and G each independently represent a halogen atom, B(OH)<sub>2</sub>, a substituent represented by the above structural formula (V-1), a substituent represented by the above structural formula (V-2), or a substituent represented by the above structural formula (V-3). Furthermore, in the formula (III), R<sup>1</sup>, Ar and n have the same meanings as R<sup>1</sup>, Ar and n in the formula (I), respectively.

Also, at the time of the above-described reaction, a metal, a metal complex catalyst, a base, a solvent or the like may be used as necessary.

As the metal, for example, palladium (Pd), copper (Cu), titanium (Ti), tin (Sn), nickel (Ni), or platinum (Pt) is used.

As the metal complex, for example, tetrakis(triphenylphosphine)palladium (Pd(PPh<sub>3</sub>)<sub>4</sub>), palladium(II) acetate (Pd(OCOCH<sub>3</sub>)<sub>2</sub>), tris(dibenzylideneacetone)ditritylpalladium(0) (Pd<sub>2</sub>(dba)<sub>3</sub>), di(triphenylphosphine)dichloropalladium (Pd(PPh<sub>3</sub>)<sub>2</sub>Cl<sub>2</sub>), 1,1'-bis(diphenylphosphino) ferrocenepalladium(II) dichloride dichloromethane complex (Pd(dppf)<sub>2</sub>Cl<sub>2</sub>), Pd/C, or nickel(II) acetylacetone (Ni(acac)<sub>2</sub>) is used.

As the base, for example, an inorganic base such as sodium carbonate (Na<sub>2</sub>CO<sub>3</sub>), potassium carbonate (K<sub>2</sub>CO<sub>3</sub>), cesium carbonate (Cs<sub>2</sub>CO<sub>3</sub>), or barium hydroxide (Ba(OH)<sub>2</sub>), or an organic base such as triethylamine (NEt<sub>3</sub>), diisopropylamine (NH(i-Pr)<sub>2</sub>), diethylamine (NHEt<sub>2</sub>), dimethylamine

an ether solvent such as diethyl ether, tetrahydrofuran or dioxane; acetonitrile, dimethylformamide, dimethyl sulfoxide, methanol, ethanol, isopropyl alcohol or water is used.

Furthermore, during the reaction, for example, triphenylphosphine (PPh<sub>3</sub>), tri-o-tolylphosphine (P(o-Tol)<sub>3</sub>), tributylphosphine (P(t-Bu)<sub>3</sub>), or triethylphosphine (PEt<sub>3</sub>) is used as necessary.

However, Me represents "CH<sub>3</sub>"; Et represents "C<sub>2</sub>H<sub>5</sub>"; Ph represents "C<sub>6</sub>H<sub>5</sub>"; i-Pr represents "(CH<sub>3</sub>)<sub>2</sub>CH<sub>2</sub>"; o-Tol represents "o-CH<sub>3</sub>C<sub>6</sub>H<sub>4</sub>"; and t-Bu represents "(CH<sub>3</sub>)<sub>3</sub>C".

The reaction described above may be carried out, for example, under normal pressure in an inert gas atmosphere of nitrogen or argon, but may also be carried out under pressurized conditions.

The reaction temperature for the reaction may be, for example, in the range of from 20° C. to 300° C., but may also be in the range of from 50° C. to 180° C. The reaction time may vary with the reaction conditions, but may be selected in the range of, for example, from 5 minutes to 20 hours.

The amount of the metal or metal complex catalyst used is not particularly limited. However, for example, the amount may be in the range of from 0.001 mole to 10 moles relative to 1 mole of the compound represented by the formula (III), and may also be in the range of from 0.01 mole to 5.0 moles.

The amount of the base used may be in the range of from 0.5 mole to 4.0 moles relative to 1 mole of the compound represented by the formula (III), and may also be in the range of from 1.0 mole to 2.5 moles.

After the reaction, a crude product is obtained by, for example, introducing the reaction solution into water, subsequently stirring the mixture, and if the reaction product is in the form of crystals, collecting the crystals through suction filtration. When the reaction product is an oily substance, a crude product is obtained by, for example, extracting the reaction product with a solvent such as ethyl acetate or toluene. The crude product thus obtained may be, for example, subjected to column purification with silica gel, alumina, activated white clay or activated carbon, or may be subjected to a treatment such as adding these adsorbents to the solution and adsorbing unnecessary components. Furthermore, when the reaction product is in the form of crystals, the reaction product may also be purified by recrystallizing the crystals from a solvent such as hexane, methanol, acetone, ethanol, ethyl acetate, or toluene.

However, the synthesis method according to the exemplary embodiment is not intended to be limited to these.

As specific examples of the compound represented by the formula (I), monomer compounds 1 to 31 (compounds from Monomer Compound No. 1 to Monomer Compound No. 31 in the following Table 1) are shown below, but the examples are not limited to these.

Meanwhile, R<sup>1</sup>, Ar and n in the monomer compounds I to 31 have the same meanings as R<sup>1</sup>, Ar and n in the formula (I), respectively.

| Monomer Compound No. | Ar | n | R <sup>1</sup>  |
|----------------------|----|---|-----------------|
| 1                    |    | 0 | CH <sub>3</sub> |
| 2                    |    | 0 | CH <sub>3</sub> |
| 3                    |    | 0 | CH <sub>3</sub> |
| 4                    |    | 0 | CH <sub>3</sub> |
| 5                    |    | 0 | CH <sub>3</sub> |
| 6                    |    | 1 | CH <sub>3</sub> |

**10**  
-continued

| Monomer Compound No. | Ar | n | R <sup>1</sup>  |
|----------------------|----|---|-----------------|
| 7                    |    | 1 | CH <sub>3</sub> |
| 8                    |    | 1 | CH <sub>3</sub> |
| 9                    |    | 1 | CH <sub>3</sub> |
| 10                   |    | 1 | CH <sub>3</sub> |
| 11                   |    | 1 | CH <sub>3</sub> |
| 12                   |    | 1 | CH <sub>3</sub> |
| 13                   |    | 1 | CH <sub>3</sub> |
| 14                   |    | 1 | CH <sub>3</sub> |
| 15                   |    | 1 | CH <sub>3</sub> |
| 16                   |    | 1 | CH <sub>3</sub> |
| 17                   |    | 1 | CH <sub>3</sub> |

**11**  
-continued

| Monomer<br>Compound<br>No. | Ar | n | R <sup>1</sup>  |
|----------------------------|----|---|-----------------|
| 18                         |    | 1 | CH <sub>3</sub> |
| 19                         |    | 1 | CH <sub>3</sub> |
| 20                         |    | 1 | CH <sub>3</sub> |
| 21                         |    | 1 | CH <sub>3</sub> |
| 22                         |    | 1 | CH <sub>3</sub> |
| 23                         |    | 1 | CH <sub>3</sub> |
| 24                         |    | 1 | CH <sub>3</sub> |

**12**  
-continued

| Monomer<br>Compound<br>No. | Ar                                                                                                                                                                                                      | n | R <sup>1</sup>  |
|----------------------------|---------------------------------------------------------------------------------------------------------------------------------------------------------------------------------------------------------|---|-----------------|
| 25                         |                                                                                                                                                                                                         | 1 | CH <sub>3</sub> |
| 10                         |                                                                                                                                                                                                         | 2 | CH <sub>3</sub> |
| 15                         |                                                                                                                                                                                                         | 2 | CH <sub>3</sub> |
| 20                         |                                                                                                                                                                                                         | 2 | CH <sub>3</sub> |
| 25                         |                                                                                                                                                                                                         | 2 | CH <sub>3</sub> |
| 30                         |                                                                                                                                                                                                         | 2 | CH <sub>3</sub> |
| 35                         |                                                                                                                                                                                                         | 2 | CH <sub>3</sub> |
| 40                         |                                                                                                                                                                                                         | 2 | CH <sub>3</sub> |
| 45                         |                                                                                                                                                                                                         | 2 | CH <sub>3</sub> |
| 50                         |                                                                                                                                                                                                         | 2 | CH <sub>3</sub> |
| 55                         | <p>&lt;Compound Containing Structural Unit Represented by<br/>Formula (II-1) (Polyester)&gt;</p> <p>The compound represented by the following formula (II-1)<br/>will be described in detail below.</p> |   |                 |
| 60                         | <p>Formula (II-1)</p> $R^2 - (O - Y^1)_m - O - \left[ \begin{array}{c} O \\    \\ C - A^1 - C \\    \\ O - (Y^1 - O)_m \end{array} \right]_p R^2$                                                       |   |                 |
| 65                         |                                                                                                                                                                                                         |   |                 |

In the formula (II-1),  $A^1$  represents a group represented by the following formula (II-2).



In the formula (II-2), Ar and n have the same meanings as Ar and n in the formula (I), respectively.

In the formula (II-1),  $Y^1$ 's each independently represent a substituted or unsubstituted divalent hydrocarbon group. 20

The divalent hydrocarbon group represented by  $Y^1$  is a dihydric alcohol residue, and is preferably an alkylene group, a (poly)ethylenoxy group, a (poly)propylenoxy group, an arylene group, a divalent heterocyclic group, or a combination thereof. 25

The divalent hydrocarbon group represented by  $Y^1$  is preferably a linking group with fewer carbon atoms, from the viewpoints of compatibility with resins and charge transportability. Specifically, the carbon number is preferably in the range of from 1 to 18, and more preferably in the range of from 1 to 6. 30

Furthermore, the divalent hydrocarbon group represented by  $Y^1$  is preferably a linking group having a smaller dipole moment from the viewpoint of charge transportability. Specifically, a linking group which does not contain any atom other than carbon atoms and hydrogen atoms (for example, an oxygen atom, a nitrogen atom, or a sulfur atom) is preferable. 35

That is, the divalent hydrocarbon group represented by  $Y^1$  40 is preferably an alkylene group having from 1 to 10 carbon atoms, or an arylene group having from 6 to 18 carbon atoms, and more preferably an alkylene group having from 1 to 6 carbon atoms.

Furthermore, as the divalent hydrocarbon group represented by  $Y^1$ , a group having smaller steric length is more preferable from the viewpoint of the compatibility with resins. Examples of the divalent hydrocarbon group having smaller steric length include a group which does not have a cyclic structure. A specific example thereof is an alkylene group having from 1 to 10 carbon atoms, and an alkylene group having from 1 to 5 carbon atoms is more preferable. Furthermore, in addition to the compatibility with resins, from the viewpoint that a polymer compound having a large molecular weight is easily synthesized, an alkylene group having 2 carbon atoms is most preferable. 45 50 55

Specifically,  $Y^1$  in the formula (II-1) may be a group selected from groups represented by the following formula (1) to formula (8).

14

(II-2)

-continued

(3) 

(4) 

(5) 

(6) 

(7) 

(8) 

In the formulae (1) and (2),  $d$  and  $e$  each independently represent an integer of from 1 to 10.

In the formulae (5) and (6),  $R^4$  and  $R^5$  each independently represent an alkyl group having from 1 to 4 carbon atoms, an alkoxy group having from 1 to 4 carbon atoms, a substituted or unsubstituted phenyl group, a substituted or unsubstituted aralkyl group, or a halogen atom.

In the formulae (5) and (6), f and g each represent an integer of 0, 1 or 2; h and i each represent 0 or 1; and V represents a group selected from groups represented by the following formula (9) to formula (29).



**15**

-continued

**16**

-continued

(28)



(29)



(13)

(14)

(15)

(16)

(17)

(18)

(19)

(20)

(21)

(22)

(23)

(24)

(25)

(26)

(27)

In the formula (9), b represents an integer of from 1 to 10, preferably represents an integer of from 1 to 6, and more preferably represents an integer of from 1 to 4.

In the formula (15), R<sup>6</sup>'s each independently represent a hydrogen atom, an alkyl group or a cyano group.

In the formulae (26) and (29), R<sup>7</sup>'s each independently represent a hydrogen atom, an alkyl group having from 1 to 10 carbon atoms, an alkoxy group having from 1 to 10 carbon atoms, a substituted or unsubstituted phenyl group, a substituted or unsubstituted aralkyl group, or a halogen atom.

In the formulae (15), (16) and (25) to (29), c's each independently represent an integer of from 0 to 10, preferably represent an integer of from 0 to 6, and more preferably represent an integer of from 1 to 3.

Plural Y<sup>1</sup>'s that are present in the compound containing the structural unit represented by the formula (II-1) may be identical with or different from each other, but from the viewpoint of manufacturability, it is preferable that Y<sup>1</sup>'s be identical.

In the formula (II-1), m represents an integer of from 1 to 5. From the viewpoint of a balance between solubility and the increase of the molecular weight, m is preferably an integer of from 1 to 3, and from the viewpoint of increasing the molecular weight, m is more preferably an integer of from 2 to 2. Furthermore, from the viewpoint of making the electrical characteristics of the image holding member for an image forming apparatus satisfactory, m in the formula (II-1) is most preferably 1.

In the formula (II-1), R<sup>2</sup>'s each independently represent a hydrogen atom, an alkyl group, a substituted or unsubstituted aryl group, or a substituted or unsubstituted aralkyl group.

Specific examples of the alkyl group, aryl group and aralkyl group, and of the substituents substituting those groups are the same as the specific examples described above as the substituents substituting the aromatic ring of Ar.

Furthermore, in the formula (II-1), R<sup>2</sup> may be a hydrogen atom or a phenyl group among those, and from the viewpoints of low cost and ease of production, R<sup>2</sup> may be a hydrogen atom. Furthermore, two R<sup>2</sup>'s in the formula (II-1) may be identical with or different from each other, but when R<sup>2</sup>'s are identical, it is easier to produce a charge transporting polyester.

Two R<sup>2</sup>'s in the formula (II-1) may be identical with or different from each other, but from the viewpoint of manufacturability, it is preferable that R<sup>2</sup>'s be identical.

In the formula (II-1), p represents an integer of from 5 to 5,000, but may also be in the range of from 10 to 1000.

More specifically, the weight average molecular weight Mw of the charge transporting polyester may be, for example, in the range of from 5,000 to 300,000, and may also be in the range of from 10,000 to 1,000,000.

The weight average molecular weight Mw is measured by the following method. That is, the weight average molecular weight is determined by preparing a 1.0% by weight tetrahydrofuran solution of a charge transporting polyester, and mea-

suring the molecular weight by gel permeation chromatography (GPC) using a differential refractive index detector (RI), while using styrene polymers as standard samples.

Furthermore, the glass transition temperature ( $T_g$ ) of the charge transporting polyester may be, for example, from 60° C. to 300° C., and may also be from 100° C. to 200° C.

Meanwhile, the glass transition temperature is measured by differential scanning calorimetry using  $\alpha$ -Al<sub>2</sub>O<sub>3</sub> as a reference, by increasing the temperature of the sample until the sample reaches a rubbery state, quenching the sample by immersing the sample in liquid nitrogen, and then increasing the temperature again under the conditions of a rate of temperature increase of 10° C./min.

<Method for Producing Compound Containing Structural Unit Represented by Formula (II-1) (Polyester)>

A compound containing the structural unit represented by the formula (II-1) (polyester) is synthesized by performing polymerization by a known method, using a compound represented by the formula (I) obtained as described above.

A specific example is a method of introducing a substituent that will be described below, to the end of R<sup>1</sup> in the formula (I), and specifically, the following synthesis methods may be used.

1) When R<sup>1</sup> is Hydroxyl Group

A compound represented by the formula (I-3) is mixed with, for example, an equivalent amount of a dihydric alcohol represented by the formula: HO—(Y<sup>1</sup>—O)<sub>m</sub>—H, and the mixture is polymerized by using an acid catalyst. Meanwhile, Y<sup>1</sup> represents a dihydric alcohol residue, and has the same meaning as Y<sup>1</sup> in the formula (II-1). m represents an integer of from 1 to 5, and has the same meaning as m in the formula (II-1).

As the acid catalyst described above, any acid catalyst used in conventional esterification reactions, such as sulfuric acid, toluenesulfuric acid or trifluoroacetic acid is used. The acid catalyst is used in an amount in the range of from 1/10,000 part by weight to 1/10 part by weight, and preferably in the range of from 1/1,000 part by weight to 1/50 part by weight, relative to 1 part by weight of the monomer (that is, the compound represented by the formula (I); hereinafter, the same).

In order to remove water that is produced during the polymerization, it is preferable to use a solvent which azeotropically boils with water. Examples of the solvent which azeotropically boils with water include toluene, chlorobenzene, and 1-chloronaphthalene, and the solvent is used in an amount in the range of from 1 part by weight to 100 parts by weight, and preferably in the range of from 2 parts by weight to 50 parts by weight, relative to 1 part by weight of the monomer.

The reaction temperature is set according to the conditions, but in order to remove water that is produced during the polymerization, it is preferable to carry out the reaction at the boiling point of the solvent.

After completion of the reaction, if a solvent has not been used in the reaction, the reaction product is dissolved in a solvent which dissolves the product. If a solvent has been used, the reaction solution is directly added dropwise to an alcohol such as methanol or ethanol, or to a poor solvent in which the polymer is not easily dissolved, such as acetone, and thereby the polyester is precipitated. The polyester is separated, and then is washed with water or an organic solvent and dried.

Furthermore, if necessary, a reprecipitation treatment of dissolving the polyester in an organic solvent, adding the solution dropwise to a poor solvent, and precipitating the polyester may be repeated. During the reprecipitation treat-

ment, it is preferable to carry out the treatment while the system is efficiently stirred with a mechanical stirrer or the like. At the time of the reprecipitation treatment, the solvent for dissolving the polyester is used in an amount in the range of from 1 part by weight to 100 parts by weight, and preferably in the range of from 2 parts by weight to 50 parts by weight, relative to 1 part by weight of the polyester. The poor solvent is used in an amount in the range of from 1 part by weight to 1,000 parts by weight, and preferably in the range of from 10 parts by weight to 500 parts by weight, relative to 1 part by weight of the polyester.

2) When R<sup>1</sup> is Halogen

A compound represented by the formula (I) is mixed with, for example, an equivalent amount of a dihydric alcohol represented by the formula: HO—(Y<sup>1</sup>—O)<sub>m</sub>—H, and the mixture is polymerized by using an organic basic catalyst such as pyridine or triethylamine. Meanwhile, Y<sup>1</sup> represents a dihydric alcohol residue, and has the same meaning as Y<sup>1</sup> in the formula (II-1). m represents an integer of from 1 to 5, and has the same meaning as m in the formula (II-1).

The organic basic catalyst is used in an amount in the range of from 1 equivalent to 10 equivalents, and preferably in the range of from 2 equivalents to 5 equivalents, relative to 1 equivalent of the monomer (that is, the compound represented by the formula (I)).

Examples of the solvent include methylene chloride, tetrahydrofuran (THF), toluene, chlorobenzene, and 1-chloronaphthalene, and the solvent is used in an amount in the range of from 1 part by weight to 100 parts by weight, and preferably in the range of from 2 parts by weight to 50 parts by weight, relative to 1 part by weight of the monomer.

The reaction conditions are set according to the conditions. After the polymerization, a reprecipitation treatment is carried out as described above, and thus the polyester is purified.

Furthermore, when a dihydric alcohol having a high degree of acidity, such as bisphenol, is used, an interfacial polymerization method may also be used. That is, polymerization is carried out by adding a dihydric alcohol to water, adding an equivalent amount of a base to dissolve the base therein, and then adding the dihydric alcohol and an equivalent amount of the monomer solution while vigorously stirring the reaction system. At this time, water is used in an amount in the range of from 1 part by weight to 1,000 parts by weight, and preferably in the range of from 2 parts by weight to 500 parts by weight, relative to 1 part by weight of the dihydric alcohol. Examples of the solvent for dissolving the monomer include methylene chloride, dichloroethane, trichloroethane, toluene, chlorobenzene, and 1-chloronaphthalene.

The reaction temperature is set according to the conditions, and in order to accelerate the reaction, a phase transfer catalyst such as an ammonium salt or a sulfonium salt may also be used. The phase transfer catalyst is used in an amount in the range of from 0.1 part by weight to 10 parts by weight, and preferably in the range of from 0.2 part by weight to 5 parts by weight, relative to 1 part by weight of the monomer.

3) When R<sup>1</sup> is —O—R<sup>9</sup>

Synthesis is carried out by adding an excess of a dihydric alcohol represented by the formula: HO—(Y<sup>1</sup>—O)<sub>m</sub>—H to a compound represented by the formula (I), and performing a transesterification reaction by heating the mixture using an inorganic acid such as sulfuric acid or phosphoric acid, a titanium alkoxide, an acetate or carbonate of calcium or cobalt, or an oxide of zinc or lead as a catalyst. Here, Y<sup>1</sup> represents a dihydric alcohol residue, and has the same meaning as Y<sup>1</sup> in the formula (II-1). m represents an integer of from 1 to 5, and has the same meaning as m used in the formula (II-1).

The dihydric alcohol is used in an amount in the range of from 2 equivalents to 100 equivalents, and preferably in the range of from 3 equivalents to 50 equivalents, relative to 1 equivalent of the monomer (compound represented by the formula (I)).

The catalyst is used in an amount in the range of from 1/10,000 part by weight to 1 part by weight, and preferably in the range of from 1/1,000 part by weight to 1/2 part by weight, relative to 1 part by weight of the monomer.

The reaction is carried out at a reaction temperature of from 200° C. to 300° C., and after completion of the transesterification reaction from  $-\text{O}-\text{R}^9$  to  $-\text{O}-(\text{Y}^1-\text{O})_m-\text{H}$ , it is preferable to perform the reaction under reduced pressure in order to accelerate polymerization through elimination of  $\text{HO}-(\text{Y}^1-\text{O})_m-\text{H}$ . Furthermore, the reaction may also be carried out by using a high boiling point solvent which azeotropically boils with  $\text{HO}-(\text{Y}^1-\text{O})_m-\text{H}$ , such as 1-chloronaphthalene, and azeotropically eliminating  $\text{HO}-(\text{Y}^1-\text{O})_m-\text{H}$  under normal pressure (under the atmospheric pressure).

Furthermore, the polyester represented by the formula (II-1) may be synthesized as follows.

In the respective cases of 1) to 3), a compound represented by the following formula (VII) is produced by adding an excess of a dihydric alcohol and carrying out the reaction. Subsequently, this compound is used instead of the monomer represented by the formula (I), and the compound is allowed to react with a divalent carboxylic acid, a divalent carboxylic acid halide or the like. Thereby, a polyester represented by the formula (II-1) is obtained.

| Polymer Compound No. | Structural No. of A <sup>1</sup> | Y <sup>1</sup>                                                  | m | R <sup>2</sup> | p  |
|----------------------|----------------------------------|-----------------------------------------------------------------|---|----------------|----|
| 1                    | 1                                | $-\text{CH}_2-\text{CH}_2-$                                     | 1 | H              | 55 |
| 2                    | 1                                | $-\text{CH}_2-\text{CH}_2-$                                     | 1 | H              | 58 |
| 3                    | 1                                | (a biphenyl ring with a methylene group in the para position)   | 1 | H              | 48 |
| 4                    | 1                                | (a cyclohexyl ring with a methylene group in the para position) | 1 | H              | 65 |
| 5                    | 1                                | (a biphenyl ring)                                               | 1 | H              | 57 |
| 6                    | 4                                | $-\text{CH}_2-\text{CH}_2-$                                     | 1 | H              | 57 |

(VII)



In the formula (VII), Ar and n have the same meanings as Ar and n in the formula (I), respectively, and Y<sup>1</sup> and m have the same meanings as Y<sup>1</sup> and m in the formula (II-1), respectively.

Meanwhile, among the synthesis methods of 1) to 3), production is easily achieved by following the synthesis method of 1) in the exemplary embodiment.

As specific examples of the polyester represented by the formula (II-1), polymer compounds 1 to 30 (that is, specific example polyesters 1 to 30) are shown below, but the exemplary embodiment is not limited to these specific examples.

Meanwhile, the number in the column of monomer (column of "Structural No. of A<sup>1</sup>") in the polymer compound corresponds to the Monomer Compound No. of the compound represented by the formula (I). In the following, specific examples (compounds) each assigned with a number, for example, the structure of A<sup>1</sup> assigned with the number 15 means a structure derived from the monomer compound 15.

Furthermore, Y<sup>1</sup>, m, p and R<sup>2</sup> in the polymer compounds have the same meanings as Y<sup>1</sup>, m, p and R<sup>2</sup> in the formula (II-1) respectively.

-continued

| Polymer Compound No. | Structural No. of A <sup>1</sup> | Y <sup>1</sup>                                                      | m | R <sup>2</sup> | p  |
|----------------------|----------------------------------|---------------------------------------------------------------------|---|----------------|----|
| 7                    | 4                                | (a cyclohexyl ring with two methyl groups in the 1 and 4 positions) | 1 | H              | 38 |
| 8                    | 4                                | (a biphenyl ring with a methylene group in the para position)       | 1 | H              | 58 |
| 9                    | 4                                | (a biphenyl ring)                                                   | 1 | H              | 74 |

| Polymer Compound No. | Structure No. of A <sup>1</sup> | Y <sup>1</sup>                     | m | R <sup>2</sup> | p  |
|----------------------|---------------------------------|------------------------------------|---|----------------|----|
| 10                   | 6                               | —(CH <sub>2</sub> ) <sub>2</sub> — | 1 | H              | 80 |
| 11                   | 6                               | —(CH <sub>2</sub> ) <sub>6</sub> — | 1 | H              | 71 |
| 12                   | 7                               | —(CH <sub>2</sub> ) <sub>2</sub> — | 1 | H              | 67 |
| 13                   | 9                               |                                    | 1 | H              | 52 |
| 14                   | 10                              | —(CH <sub>2</sub> ) <sub>6</sub> — | 1 | H              | 56 |
| 15                   | 12                              | —(CH <sub>2</sub> ) <sub>2</sub> — | 1 | H              | 69 |
| 16                   | 14                              | —(CH <sub>2</sub> ) <sub>2</sub> — | 1 | H              | 71 |
| 17                   | 14                              |                                    | 1 | H              | 58 |
| 18                   | 15                              | —(CH <sub>2</sub> ) <sub>2</sub> — | 1 | H              | 49 |
| 19                   | 15                              | —(CH <sub>2</sub> ) <sub>6</sub> — | 1 | H              | 61 |
| 20                   | 17                              | —(CH <sub>2</sub> ) <sub>2</sub> — | 1 | H              | 57 |
| 21                   | 18                              | —(CH <sub>2</sub> ) <sub>2</sub> — | 1 | H              | 68 |
| 22                   | 19                              | —(CH <sub>2</sub> ) <sub>2</sub> — | 1 | H              | 68 |
| 23                   | 23                              | —(CH <sub>2</sub> ) <sub>2</sub> — | 1 | H              | 83 |
| 24                   | 23                              |                                    | 1 | H              | 58 |
| 25                   | 24                              |                                    | 1 | H              | 74 |
| 26                   | 25                              | —(CH <sub>2</sub> ) <sub>2</sub> — | 1 | H              | 62 |
| 27                   | 26                              | —(CH <sub>2</sub> ) <sub>2</sub> — | 1 | H              | 59 |
| 28                   | 27                              | —(CH <sub>2</sub> ) <sub>2</sub> — | 1 | H              | 61 |
| 29                   | 28                              | —(CH <sub>2</sub> ) <sub>2</sub> — | 1 | H              | 59 |
| 30                   | 30                              | —(CH <sub>2</sub> ) <sub>6</sub> — | 1 | H              | 71 |

In the image holding member for an image forming apparatus of the exemplary embodiment, as described above, at least one of the compound represented by the formula (I) and

the compound represented by the formula (II-1) is included in the photosensitive layer. It can be contemplated that when at least one of the compound represented by the formula (I) and the compound represented by the formula (II-1) has high charge transportability, the charge injectability (particularly, injectability of positive charge) from the charge generating layer is improved. It is thought that, as a result, for example, the charge-up phenomenon and the like do not easily occur, the variance of the residual potential due to repeated use is decreased, and thus excellent environmental sustainability is exhibited.

Furthermore, in the image holding member for an image forming apparatus of the exemplary embodiment, since at least one of the compound represented by the formula (I) and the compound represented by the formula (II-1) has excellent compatibility with resins, the thickness irregularity of the photosensitive layer is decreased. It is thought that, as a result, the variance of the residual potential due to a repeated use of the image holding member is decreased.

Furthermore, in the image forming apparatus and process cartridge of the exemplary embodiment, since the image holding member for an image forming apparatus of the exemplary embodiment is used, satisfactory image quality may be obtained for a long time, which leads to a reduction in the environmental burden and a large cost reduction.

**<Configuration of Image Holding Member for Image Forming Apparatus>**

Hereinafter, the configuration of the image holding member for an image forming apparatus of the exemplary embodiment will be described.

The image holding member for an image forming apparatus of the exemplary embodiment is an image holding member for an image forming apparatus having a photosensitive layer on a support, and is characterized in that the photosensitive layer contains at least one of the compound represented by the formula (I) and the compound represented by the formula (II-1).

FIG. 1 to FIG. 3 are schematic cross-sectional diagrams showing the first exemplary embodiment to the third exemplary embodiment of the image holding member for an image forming apparatus of the exemplary embodiment of the present invention.

These diagrams all show the cross-sections produced by cutting the image holding member 1 for an image forming apparatus along the lamination direction of the conductive support 2 and the photosensitive layer 3.

The image holding members 1 for image forming apparatuses according to the first and second exemplary embodiments as shown in FIG. 1 and FIG. 2 include a functionally separated photosensitive layer in which a charge generating material and a charge transporting material are included in different layers. That is, in the photosensitive layer 3, a layer containing a charge generating material (charge generating layer 5) and a layer containing a charge transporting material (charge transport layer 6) are separately formed, and the layers are laminated to be adjacent to each other.

On the other hand, the image holding member 1 for an image forming apparatus according to the third exemplary embodiment as shown in FIG. 3 includes a single-layer type photosensitive layer in which a charge generating material and a charge transporting material are included in the same layer. That is, in the photosensitive layer 3, a charge generating/transport layer 8 containing a charge generating material and a charge transporting material is formed as a single layer.

More particularly, in the image holding member 1 for an image forming apparatus according to the first exemplary embodiment, an undercoat layer 4, a charge generating layer

5 and a charge transport layer 6 are laminated in this order on a conductive support 2, and thereby a photosensitive layer 3 is constructed. In the image holding member 1 for an image forming apparatus according to the second exemplary embodiment, an undercoat layer 4, a charge generating layer 5, a charge transport layer 6 and a protective layer 7 are laminated in this order on a conductive support 2, and thereby a photosensitive layer 3 is constructed. Furthermore, in the image holding member 1 for an image forming apparatus according to the third exemplary embodiment, an undercoat layer 4 and a charge generating/transport layer 8 are laminated in this order on a conductive support 2, and thereby a photosensitive layer 3 is constructed.

Although not depicted in the diagrams, as a modification of the second exemplary embodiment, an embodiment in which the lamination sequence of the charge generating layer 5 and the charge transport layer 6 of the second exemplary embodiment is inverted, or as a modification of the third exemplary embodiment, an embodiment in which the protective layer 7 used in the second exemplary embodiment is formed on the charge generating/transport layer 8 of the third exemplary embodiment, may also be used.

As the conductive support 2, a support produced by forming aluminum into a drum shape, a sheet shape, a plate shape or the like may be used, but the conductive support is not intended to be limited to these. The conductive support 2 may be subjected to an anodization treatment, a boehmite treatment, a honing treatment or the like.

In the region interposed between the conductive support 2 and the photosensitive layer 3 or the region interposed between the conductive support 2 and the charge generating/transport layer 8, as shown in FIG. 1 to FIG. 3, the undercoat layer 4 is provided. The undercoat layer 4 is formed by using an organozirconium compound such as a zirconium chelate compound, a zirconium alkoxide compound, or a zirconium coupling agent; an organotitanium compound such as a titanium chelate compound, a titanium alkoxide compound or a titanate coupling agent; an organoaluminum compound such as an aluminum chelate compound, or an aluminum coupling agent; or an organometallic compound such as an antimony alkoxide compound, a germanium alkoxide compound, an indium alkoxide compound, an indium chelate compound, a manganese alkoxide compound, a manganese chelate compound, a tin alkoxide compound, a tin chelate compound, an aluminum silicon alkoxide compound, an aluminum titanium alkoxide compound, or an aluminum zirconium alkoxide compound. Particularly, an organozirconium compound, an organotitanium compound or an organoaluminum compound is preferably used.

Furthermore, a silane coupling agent such as vinyltrichlorosilane, vinyltrimethoxysilane, vinyltriethoxysilane, vinyl-tris-2-methoxyethoxysilane, vinyltriacetoxysilane,  $\gamma$ -glycidoxypyropyltrimethoxysilane,  $\gamma$ -methacryloxypropyltrimethoxysilane,  $\gamma$ -aminopropyltriethoxysilane,  $\gamma$ -chloropropyltrimethoxysilane,  $\gamma$ -2-aminoethylaminopropyltrimethoxysilane,  $\gamma$ -mercaptopropyltrimethoxysilane,  $\gamma$ -ureidopropyltriethoxysilane, or  $\beta$ -3,4-epoxycyclohexyltrimethoxysilane is further incorporated.

Furthermore, a known binder resin such as a polyvinyl alcohol, a polyvinyl methyl ether, a poly-N-vinylimidazole, a polyethylene oxide, an ethyl cellulose, a methyl cellulose, an ethylene-acrylic acid copolymer, a polyamide, a polyimide, casein, gelatin, a polyethylene, a polyester, a phenolic resin, a vinyl chloride-vinyl acetate copolymer, an epoxy resin, a polyvinylpyrrolidone, a polyvinylpyridine, a polyurethane, a

polyglutamic acid, or a polyacrylic acid may be further incorporated. The mixing proportions of these agents may be set according to necessity.

Furthermore, in the undercoat layer 4, an electron transporting pigment may be used by mixing or dispersing the pigment in the layer.

Examples of the electron transporting pigment include organic pigments such as the perylene pigments, bisbenzimidazole perylene pigments, polycyclic quinone pigments, 10 indigo pigments, and quinacridone pigments described in JP-A-47-30330. Furthermore, organic pigments such as bisazo pigments having electron-withdrawing substituents such as a cyano group, a nitro group, a nitroso group or a halogen atom, and phthalocyanine pigments; and inorganic 15 pigments such as zinc oxide and titanium oxide may be used. Among these pigments, a perylene pigment, a bisbenzimidazole perylene pigment, a polycyclic quinone pigment, zinc oxide or titanium oxide is preferable.

Furthermore, the surfaces of these pigments may be 20 surface treated with the coupling agents described above, or with binders. The content of the electron transporting pigment used in the undercoat layer 4 is 95% by weight or less, and preferably 90% by weight or less, relative to the total weight of the undercoat layer 4.

25 As the method for mixing or dispersing an electron transporting pigment in the undercoat layer 4, routine methods of using a ball mill, a roll mill, a sand mill or an attritor, or using ultrasonic waves are applied. The process of mixing and dispersing is carried out in an organic solvent, and as the 30 organic solvent, any solvent which is capable of dissolving an organometallic compound or a resin, and does not cause gelation or aggregation when an electron transporting pigment is mixed or dispersed therein, may be used.

The thickness of the undercoat layer 4 is preferably from 35 0.1  $\mu$ m to 30  $\mu$ m, and more preferably from 0.2  $\mu$ m to 25  $\mu$ m.

Furthermore, as the coating method used to provide the undercoat layer 4, a conventional method such as a blade coating method, a Meyer bar coating method, a spray coating method, a dip coating method, a bead coating method, an air 40 knife coating method, or a curtain coating method is used.

A coating film formed by applying a composition for undercoat layer formation containing the above-described components is dried to thereby obtain an undercoat layer 4, and usually, the drying process is carried out at a temperature 45 at which a film may be formed by evaporating the solvent. Particularly, since a base material that has been subjected to an acidic solution treatment or a boehmite treatment is likely to have an insufficient defect covering power of the base material, it is preferable to form the undercoat layer 4.

50 As the charge generating material incorporated in the charge generating layer 5, well known materials such as azo pigments such as bisazo and trisazo compounds; condensed ring aromatic pigments such as dibromoanthanthrone; perylene pigments, pyrrolopyrrole pigments, and phthalocyanine pigments may be used, but particularly, metallic and metal-free phthalocyanine pigments are preferable. Among them, hydroxygallium phthalocyanine disclosed in JP-A-5-263007 and JP-A-5-279591; chlorogallium phthalocyanine disclosed in JP-A-5-98181; dichlorotin phthalocyanine disclosed in JP-A-5-140472 and JP-A-5-140473; or titanyl phthalocyanine disclosed in JP-A-4-189873 and JP-A-5-43813 is particularly preferable.

55 The charge generating layer 5 is formed by mixing a charge generating material and a binder resin, and such a binder resin is selected from a wide variety of insulating resins, and may also be selected from organic photoconductive polymers such as poly-N-vinylcarbazole, polyvinylanthracene, polyvi-

nylpyrene, and polysilanes. Preferable examples of the binder resin include, but are not limited to, insulating resins such as a polyvinyl butyral resin, a polyallylate resin (a polycondensate of bisphenol A and phthalic acid, or the like), a polycarbonate resin, a polyester resin, a phenoxy resin, a vinyl chloride-vinyl acetate copolymer, a polyamide resin, an acrylic resin, a polyacrylamide resin, a polyvinylpyridine resin, a cellulose resin, a urethane resin, an epoxy resin, casein, a polyvinyl alcohol resin, and a polyvinylpyrrolidone resin. These binder resins are used individually or as mixtures of two or more kinds thereof.

Furthermore, the insulating resin as used in the exemplary embodiment refers to an insulating resin having a volume resistivity of  $10^{12} \Omega \cdot \text{cm}$  or higher as measured based on JIS K 7194 "Testing method for resistivity of conductive plastics with a four-point probe array".

The mixing ratio (weight ratio) of the charge generating material and the binder resin is preferably in the range of 10:1 to 1:10, and more preferably 8:3 to 3:8.

Furthermore, as a method of dispersing these components, a conventional method such as a ball mill dispersion method, an attritor dispersion method, or a sand mill dispersion method is used, but at this time, conditions under which the crystal form of the charge generating material will not change as a result of dispersing are required. Meanwhile, it is confirmed that the above-described dispersing methods used in the exemplary embodiment are not changed in the crystal form as compared with the crystal form before the dispersing process.

Furthermore, during this dispersion, it is effective to adjust the particles of the charge generating material to a particle size of 0.5  $\mu\text{m}$  or less, preferably 0.3  $\mu\text{m}$  or less, and more preferably 0.15  $\mu\text{m}$  or less.

The thickness of the charge generating layer 5 is preferably from 0.1  $\mu\text{m}$  to 5  $\mu\text{m}$ , and more preferably from 0.2  $\mu\text{m}$  to 2.0  $\mu\text{m}$ . Furthermore, as the coating method used to provide the charge generating layer 5, a conventional method such as a blade coating method, a Meyer bar coating method, a spray coating method, a dip coating method, a bead coating method, an air knife coating method, or a curtain coating method is used.

As the charge transport layer 6, any layer formed by a known technology may be used, except for incorporating at least one of the compound represented by the formula (I) and the compound represented by the formula (II-1).

The charge transport layer 6 is such that as long as at least one of the compound represented by the formula (I) and the compound represented by the formula (II-1) is incorporated, the charge transport layer 6 may be formed to additionally contain a charge transporting material, a binder resin or the like. Meanwhile, in the case where the compound represented by the formula (I) is used so that the compound represented by the formula (II-1) is not used, it is preferable to use the compound represented by the formula (I) by dispersing the compound in a binder resin or the like. Furthermore, in the case of using the compound represented by the formula (II-1), the charge transport layer 6 is formed even without using other resins; however, from the viewpoint of cost reduction, it is preferable to use the compound represented by the formula (II-1) in a mixture with other resins.

Examples of other charge transporting materials include other charge transporting materials, including electron transporting compounds, such as quinone-based compounds such as p-benzoquinone, chloranil, bromanil, and anthraquinone, tetracyanoquinodimethane-based compounds, fluorenone compounds such as 2,4,7-trinitrofluorenone, xanthone-based compounds, benzophenone-based compounds, cyanovinyl-

based compounds, and ethylene-based compounds; and hole transporting compounds such as triarylamine-based compounds, benzidine-based compounds, arylalkane-based compounds, aryl-substituted ethylene-based compounds, stilbene-based compounds, anthracene-based compounds, and hydrazone-based compounds. However, the charge transporting materials are not limited to these.

The content of the compound represented by the formula (I) and the compound represented by the formula (II-1) in the total amount of the charge transport layer 6 is preferably from 5% by weight to 70% by weight, more preferably from 10% by weight to 60% by weight, and even more preferably from 20% by weight to 50% by weight.

When the compound represented by the formula (I) and the compound represented by the formula (II-1) are used in combination as the charge transporting material, the content of the compound represented by the formula (I) and the compound represented by the formula (II-1) in the total amount of the charge transporting material is preferably 1% by weight or more, and more preferably 5% by weight or more.

In the case of using a binder resin in the charge transporting layer 6, examples of the binder resin include polymeric charge transporting materials such as a polycarbonate resin, a polyester resin, a methacrylic resin, an acrylic resin, a polyvinyl chloride resin, a polyvinylidene chloride resin, a polystyrene resin, a polyvinyl acetate resin, a styrene-butadiene copolymer, a vinylidene chloride-acrylonitrile copolymer, a vinyl chloride-vinyl acetate-maleic anhydride copolymer, a silicone resin, a silicone-alkyd resin, a phenol-formaldehyde resin, a styrene-alkyd resin, poly-N-vinylcarbazole, polysilane, and the polyester-based polymeric charge transporting material disclosed in JP-A-8-176293 or JP-A-8-208820. These binder resins are used individually or as mixtures of two or more kinds thereof. The mixing ratio of (weight ratio) of the charge transporting material and the binder resin is preferably 10:1 to 1:10, and more preferably 8:3 to 3:8.

The thickness of the charge transport layer 6 is preferably from 5  $\mu\text{m}$  to 50  $\mu\text{m}$ , and more preferably from 10  $\mu\text{m}$  to 30  $\mu\text{m}$ .

As the coating method, a conventional method such as a blade coating method, a wire bar coating method, a spray coating method, a dip coating method, a bead coating method, an air knife coating method, or a curtain coating method is used.

Furthermore, additives such as an antioxidant, a light stabilizer and a thermal stabilizer may be added to the photosensitive layer.

Also, the photosensitive layer may contain at least one electron accepting material.

The image holding member for an image forming apparatus of the exemplary embodiment may include a protective layer 7 (surface layer), and it is preferable to make the protective layer 7 as a high-strength protective layer (high-strength surface layer). As this high-strength protective layer, a layer in which conductive particles are dispersed in a binder resin, a layer in which lubricating particles of a fluoro resin, an acrylic resin or the like are dispersed in a conventional charge transport layer material, or a hard coating agent formed from a silicone or an acrylic resin, is used. The high-strength protective layer preferably contains a siloxane-based resin which has charge transporting properties and has a crosslinked structure.

In the protective layer 7, other coupling agents and fluorine compounds may be incorporated. Various silane coupling agents and commercially available silicone-based hard coating agents are used as these compounds.

The coating liquid used in the formation of the protective layer 7 may be prepared without solvent, or may be prepared using a solvent as necessary.

The reaction temperature and time may vary with the type of the raw material, but usually, the reaction is carried out at a temperature of from 0° C. to 100° C., preferably from 10° C. to 70° C., and particularly preferably from 15° C. to 50° C. The reaction time is not particularly limited, but the reaction time is preferably in the range of from 10 minutes to 100 hours.

Examples of a curing catalyst include a protic acid such as hydrochloric acid, acetic acid, phosphoric acid or sulfuric acid; a base such as ammonia or triethylamine; an organotin compound such as dibutyltin diacetate, dibutyltin dioctoate, or stannous octoate; an organotitanium compound such as tetra-n-butyl titanate or tetraisopropyl titanate; an organoaluminum compound such as aluminum tributoxide or aluminum triacetylacetone; an iron salt, a manganese salt, a cobalt salt, a zinc salt or a zirconium salt of an organic carboxylic acid. However, a metal compound is preferable, and a metal acetylacetone or a metal acetylacetate is more preferable, while aluminum triacetylacetone is particularly preferable.

The amount of the curing catalyst used is set according to necessity, but the amount is preferably from 0.1% by weight to 20% by weight, and more preferably from 0.3% by weight to 10% by weight, relative to the total amount of the material containing a hydrolyzable silicon substituent.

The curing temperature is set according to necessity, but in order to obtain a desired strength, the curing temperature is set to a temperature of 60° C. or higher, and more preferably 80° C. or higher. The curing time is set according to necessity, but the curing time is preferably from 10 minutes to 5 hours.

Furthermore, after the curing reaction is carried out, it is also effective to maintain the protective layer in a high humidity state. Also, depending on the use, the protective layer is hydrophobized by performing a surface treatment using hexamethyldisilazane, trimethylchlorosilane or the like.

In the protective layer 7 of the image holding member for an image forming apparatus, it is preferable to add an antioxidant.

Furthermore, in the protective layer 7 of the image holding member for an image forming apparatus, a resin which dissolves in alcohol may also be added.

Also, various particles may also be added to the protective layer 7. The particles may be used individually, but may also be used in combination. Examples of the particles include silicon-containing particles, fluorine-based particles and semiconductive metal oxide particles.

The protective layer 7 may also contain oil such as a silicone oil.

In the case of a single-layer type photosensitive layer, the single-layer type photosensitive layer may be formed to contain the charge generating material described above, the charge transporting material described above (including at least one of the compound represented by the formula (I) and the compound represented by the formula (II-1) of the exemplary embodiment), and a binder resin. Meanwhile, the charge transporting material may include a polymeric charge transporting material. As the binder resin, those listed as the binder resin used in the charge generating layer 5 and the charge transport layer 6 are used. The content of the charge generating material in the single-layer type photosensitive layer is from 10% by weight to 85% by weight, and preferably from 20% by weight to 50% by weight. Also, the content of

the charge transporting material in the single-layer type photosensitive layer is preferably from 5% by weight to 50% by weight.

As the solvent or coating method used in the coating of the layer, the solvents and coating methods described above are used. The thickness of the single-layer photosensitive layer is preferably from 5  $\mu\text{m}$  to 50  $\mu\text{m}$ , and more preferably from 10  $\mu\text{m}$  to 40  $\mu\text{m}$ .

(Image Forming Apparatus)

10 The image forming apparatus of the exemplary embodiment of the present invention is characterized by including the image holding member for an image forming apparatus of the exemplary embodiment described above; a charging unit that charges the image holding member for an image forming apparatus; an exposure unit that exposes the charged image holding member for an image forming apparatus to form an electrostatic latent image; a developing unit that develops the electrostatic latent image to form a toner image; and a transfer unit that transfers the toner image to a transfer medium.

15 FIG. 4 is a cross-sectional diagram schematically showing the basic configuration of a suitable exemplary embodiment of the image forming apparatus of the exemplary embodiment of the present invention.

20 The image forming apparatus 200 shown in FIG. 4 includes the image holding member 207 for an image forming apparatus of the exemplary embodiment of the present invention; a charging unit 208 that charges the image holding member 207 for an image forming apparatus by a contact charging mode; a power supply 209 that is connected to the charging unit 208; an exposure unit 210 that exposes the image holding member 207 for an image forming apparatus charged by the charging unit 208 to form an electrostatic latent image; a developing unit 211 that develops the electrostatic latent image formed by the exposure unit 210 with a toner to form a toner image; a transfer unit 212 that transfers the toner image formed by the developing unit 211 to a transfer medium 500; a cleaning unit 213; an erasing device 214; and a fixing unit 215.

25 The charging unit 208 shown in FIG. 9 brings a contact type charging member (for example, a charging roller) into contact with the surface of the image holding member 207 for an image forming apparatus, and charges the surface of the image holding member by applying a voltage to the image holding member.

30 As the contact type charging member, a roller-shaped member provided with an elastic layer, a resistive layer, a protective layer and the like on the outer peripheral surface of a core material, is suitably used. The shape of the contact type charging member may be any of a brush shape, a blade shape or a pin electrode shape, in addition to the roller shape described above, and the shape is selected in accordance with the specifications or form of the image forming apparatus.

35 As the material of the core material for the roller-shaped contact type charging member, a material having electrical conductivity, for example, iron, copper, brass, stainless steel, aluminum, or nickel is used. Furthermore, a resin-molded article containing dispersed conductive particles, or the like is used. As the material of the elastic layer, a material having electrical conductivity or semiconductivity, for example, a rubber material having conductive particles or semiconductive particles dispersed therein is used. As the material of the resistive layer and the protective layer, a binder resin having its resistance controlled by dispersing conductive particles or semiconductive particles therein, is used.

40 45 50 55 60 65 When the image holding member is charged by using such a contact type charging member, a voltage is applied to the contact type charging member, but the voltage applied as such

may be any of a direct current voltage, and an alternating current voltage superimposed on a direct current voltage.

Meanwhile, a corona charging unit of an on-contact system, such as a corotron or a scorotron, may also be used instead of the contact type charging member shown in FIG. 4. This is selected in accordance with the specifications or form of the image forming apparatus.

As the exposure unit 210, an optical device which exposes the surface of the image holding member for an image forming apparatus imagewise as desired to a light source such as a semiconductor laser, a light emitting diode (LED), or a liquid crystal shutter, may be used.

As the developing unit 211, a conventionally known developing unit using a regular or reversal developer of a single-component system or a two-component system, may be used. The shape of the toner used in the developing unit 211 is not particularly limited, but a spherical toner is preferable.

As the transfer unit 212, a contact type transfer charger using a belt, a film, a rubber blade or the like, or a scorotron transfer charger or corotron transfer charger using corona discharge may be used, in addition to the roller-shaped contact charging member.

The cleaning unit 213 is intended to remove any residual toner adhering to the surface of the image holding member for an image forming apparatus after the transfer step, and the image holding member for an image forming apparatus having its surface cleaned thereby may be repeatedly supplied to the image forming process. As the cleaning unit, brush cleaning, roll cleaning or the like is used, in addition to the cleaning blade; however, among these, it is preferable to use a cleaning blade. Furthermore, examples of the material of the cleaning blade include a urethane rubber, a neoprene rubber, and a silicone rubber.

The exemplary embodiment described above has one image forming unit, but an image forming apparatus according to another exemplary embodiment is a tandem type image forming apparatus having plural image forming units.

For example, when there are four image forming units, in the respective developing apparatuses of the four image forming units, for example, color component toners of four colors such as yellow, magenta, cyan and black are used. Also, it is preferable that a tandem type image forming apparatus include, commonly in the four image forming units, a belt that conveys a recording material, a conveying unit that conveys this belt, a toner supply unit that supplies a toner image to the respective developing apparatuses, and a fixing unit that fixes a color toner image to a recording material.

Furthermore, when the image holding member is used repeatedly for 200,000 cycles or more, or for 250,000 cycles or more, or even for 300,000 cycles or more, it is preferable that the image forming apparatus of the exemplary embodiment have a mechanism which replenishes only the toners.

(Process Cartridge)

The process cartridge of the exemplary embodiment is characterized by having at least the image holding member for an image forming apparatus of the exemplary embodiment described above, and including at least one selected from a charging unit that charges the image holding member for an image forming apparatus, an exposure unit that exposes the charged image holding member for an image forming apparatus to form an electrostatic latent image, a developing unit that develops the electrostatic latent image to form a toner image, a transfer unit that transfers the toner image to a transfer medium, and a cleaning unit that cleans the image holding member for an image forming apparatus.

FIG. 5 is a cross-sectional diagram schematically showing the basic configuration of a suitable exemplary embodiment

of a process cartridge that includes the image holding member for an image forming apparatus of the exemplary embodiment.

The process cartridge 300 is a cartridge in which the image holding member 207 for an image forming apparatus is combined and integrated with a charging unit 208, a developing unit 211, a cleaning unit 213, an aperture 218 for exposure, and an aperture 217 for erasing exposure, using a mounting rail 216.

Also, this process cartridge 300 is a member configured to be detachable from the main body of the image forming apparatus which is composed of a transfer unit 212 that transfers the toner image formed by the developing unit 211 to a transfer medium 500, a fixing unit 215, and other constituent parts that are not shown in the diagram, and the process cartridge constitutes an image forming apparatus together with the main body of the image forming apparatus.

Thus, the exemplary embodiment of the present invention has been explained, but the exemplary embodiment may include various alterations or modifications within the scope of the gist of the invention.

## EXAMPLES

Hereinafter, the present invention will be described based on Examples, but the invention is not intended to be limited to these.

Furthermore, in the Examples of the present invention, <sup>1</sup>H-NMR spectroscopy (solvent: CDCl<sub>3</sub>, manufactured by Varian, Inc., UNITY-300, 300 MHz) and infrared (IR) spectroscopy (Fourier transformed infrared spectrophotometer using the KBr method, manufactured by Horiba, Ltd., FT-730, resolution power 4 cm<sup>-1</sup>) are used for the identification of the target substance.

Furthermore, in the Examples, the molecular weight of a polymer is measured by gel permeation chromatography (GPC) (manufactured by Tosoh Corp., HLC-8120GPC).

### Synthesis of Compound Represented by Formula (I) or (II-1)

#### Synthesis Example 1

#### Synthesis of Monomer Compound 6

Acetanilide (25.0 g), methyl 4-iodophenylpropionate (64.4 g), potassium carbonate (38.3 g), copper sulfate pentahydrate (2.3 g), and n-tridecane (50 ml) are introduced into a 500-ml three-necked flask, and the mixture is heated and stirred for 20 hours at 230° C. under a nitrogen gas stream.

After completion of the reaction, potassium hydroxide (15.6 g) dissolved in ethylene glycol (300 ml) is added to the flask, and the mixture is heated to reflux for 3.5 hours under a nitrogen gas stream. Subsequently, the reaction liquid is cooled to room temperature (25° C.), and the reaction liquid is poured into 1 L of distilled water and is neutralized with hydrochloric acid. Thus, crystals are precipitated out. The crystals are filtered by suction filtration, washed with water, and then transferred into a 1-L flask. Toluene (500 ml) is added to these crystals, and the mixture is heated to reflux. Water is removed by azeotropically boiling the mixture, and then a methanol (300 ml) solution of concentrated sulfuric acid (1.5 ml) is added thereto. The resulting mixture is heated to reflux for 5 hours under a nitrogen gas stream.

After the reaction, the mixture is extracted with toluene, and the organic layer is washed with pure water. Subsequently, the organic layer is dried over anhydrous sodium

31

sulfate, subsequently the solvent is distilled off under reduced pressure, and the product is recrystallized from hexane. Thereby, 36.5 g of DAA-1 is obtained.



Next, a liquid mixture of 1-bromo-4-iodobenzene (5.3 g), DAA-1 (5.0 g), copper (II) sulfate pentahydrate (0.2 g), potassium carbonate (1.3 g), and tridecane (10 ml) is stirred for 6 hours at 210° C.

After completion of the reaction, potassium hydroxide (15.6 g) dissolved in ethylene glycol (300 ml) is added to the reaction liquid, and the mixture is heated to reflux for 3.5 hours under a nitrogen gas stream. Subsequently, the reaction liquid is cooled to room temperature (25° C.), and the reaction liquid is poured into 1 L of distilled water and is neutralized with hydrochloric acid. Thus, crystals are precipitated out. The crystals are filtered by suction filtration, and are washed with water, and then are transferred into a 1-L flask. Toluene (500 ml) is added to these crystals, and the mixture is heated to reflux. Water is removed by azeotropically boiling the mixture, and then a methanol (300 ml) solution of concentrated sulfuric acid (1.5 ml) is added thereto. The resulting mixture is heated to reflux for 5 hours under a nitrogen gas stream.

The mixture is cooled to room temperature (25° C.), toluene is added thereto, and the mixture is filtered through Celite. The mixture is washed with pure water, the organic layer is extracted, and the organic solvent is distilled off. A product thus obtained is separated by silica gel column chromatography (hexane 4:toluene 1), and thus 4.5 g of TAA-1 is obtained.



32

-continued



15 Next, in a 500-ml three-necked flask, 30% aqueous hydrogen peroxide (34.0 g) is added dropwise to a mixture of dibenzothiophene (18.4 g) and acetic acid (200 ml) over 20 minutes, and the resultant is magnetically stirred for 9 hours at 90° C.

20 After completion of the reaction, the reaction mixture is introduced into ice bath (600 ml), and is extracted with chloroform (800 ml). The organic layer is sequentially washed with water (200 ml), a saturated aqueous solution of iron sulfate (80 ml), 10% sodium carbonate (100 ml), water (200 ml), and saturated brine (200 ml), and the product is dried over calcium chloride. The organic solvent is distilled off, and thus colorless crystals are obtained. These are subjected to recrystallization (chloroform 150 ml, ethanol 200 ml), and thus 18.2 g of dibenzothiophene dioxide is obtained.



40 In a 500-ml three-necked flask, dibenzothiophene dioxide (18 g) is dissolved in sulfuric acid (250 ml), and N-bromosuccinimide (29.6 g) is added thereto. The mixture is stirred for 18 hours at room temperature (25° C.), and then the reaction solution is slowly introduced into ice water (800 ml). A precipitate generated therefrom is suction filtered, and the precipitate is washed with water (200 ml), a 10% aqueous NaOH solution (100 ml), and water (200 ml) and dried over calcium chloride. The precipitate is recrystallized with chloroform (700 ml), and thus 20.1 g of 3,7-dibromodibenzothiophene dioxide is obtained.



65 In a 500-ml flask, lithium aluminum hydride (4.1 g) is slowly introduced in small amounts over 50 minutes into a mixture of 3,7-dibromodibenzothiophene dioxide (20 g) and

33

anhydrous ether (200 ml) in an ice bath, and the resulting mixture is refluxed and stirred for 2 hours. Water (200 ml) is added thereto to deactivate lithium aluminum hydride. Chloroform (200 ml) and concentrated hydrochloric acid (40 ml) are added thereto, the mixture is thoroughly stirred, and the organic layer is separated. The aqueous layer is further extracted with chloroform (200 ml×2), the chloroform extract is combined with the organic layer, and the combined organic layer is washed with water (200 ml) and saturated brine (200 ml), and dried over calcium chloride. The solvent is distilled off, and colorless crystals thus obtained are recrystallized from ethyl acetate+ethanol (16:3). Thus, 8.8 g of 3,7-dibromodibenzothiophene is obtained.



34

In a nitrogen atmosphere, 3,7-dibromodibenzothiophene (8 g) is introduced into a 500-ml flask, and anhydrous tetrahydrofuran (200 ml) is added thereto to dissolve the compound. The solution is cooled to -78° C. 1.5 M tert-butyllithium (37.8 ml) is slowly added dropwise thereto over 20 minutes, and the mixture is magnetically stirred for 6 hours at -78° C. Triisopropyl borate (31.2 ml) is introduced into the flask all at once, and the content of the flask is magnetically stirred for 0.5 hours at -78° C. and is further magnetically stirred for another one hour at room temperature (25° C.). The reaction mixture is cooled to -78° C., and 1 M hydrochloric acid (100 ml) is introduced all at once. Thereafter, the reaction mixture is magnetically stirred for one hour at room temperature (25° C.) Tetrahydrofuran is distilled off, and a precipitate generated therefrom is suction filtered and dissolved in a 5% aqueous KOH solution (100 ml). 1 M hydrochloric acid is added to this solution, and a precipitate generated therefrom is suction filtered. This precipitate is dissolved in tetrahydrofuran (300 ml), 2,2-dimethyl-1,3-propanediol (4.5 g), sodium sulfate and a molecular sieve powder are added thereto to dry the precipitate. The solvent is distilled off, and the colorless crystals thus obtained are recrystallized from hexane+ethyl acetate. Thus, 4.9 g of a diboronic acid compound is obtained.



In a nitrogen atmosphere, tetrahydrofuran (250 ml) is added to tetra(triphenylphosphine)palladium (0.54 g) and TAA-1 (8.1 g) in a 500-ml flask, and the mixture is stirred for 10 minutes. Subsequently, a 2 M aqueous solution of sodium carbonate (24.5 ml) and the diboronic acid compound (2.00 g) are added, and the mixture is refluxed and magnetically stirred for 7 hours.

After completion of the reaction, ethyl acetate (100 ml) and water (50 ml) are added thereto, and the mixture is thoroughly shaken to separate an organic layer and an aqueous layer. The aqueous layer is extracted with ethyl acetate (100 ml), and the respective organic layers are washed with saturated brine (100 ml) and dried over sodium sulfate. This organic layer is separated by silica gel column chromatography (ethyl acetate/hexane=1/3), and thus 1.2 g of a monomer compound 6 is obtained.



35

36

-continued



It is confirmed by a  $^1\text{H-NMR}$  spectroscopic analysis and an IR spectroscopic analysis that the compound thus obtained is monomer compound 6.

Synthesis Example 2

Synthesis of Polymer Compound 10

1.0 g of the monomer compound 6 thus obtained, 10 ml of ethylene glycol and 0.02 g of tetrabutoxytitanium are introduced into a 50-ml three-necked pear-shaped flask, and in a nitrogen atmosphere, the mixture is heated and stirred for 5 hours at  $200^\circ\text{C}$ .

After it is confirmed by thin layer chromatography (TLC) that the raw material monomer compound 6 has reacted and disappeared, the reaction mixture is heated to  $210^\circ\text{C}$ . while ethylene glycol is distilled off by lowering the pressure to 50 Pa, and the reaction is continued for 6 hours.

Thereafter, the reaction mixture is cooled to room temperature ( $25^\circ\text{C}$ ), and is dissolved in 50 ml of tetrahydrofuran. Insoluble substances are filtered through a 0.5- $\mu\text{m}$  polytetrafluoroethylene (PTFE) filter, and the filtrate is distilled off under reduced pressure. The residue is dissolved in 300 ml of monochlorobenzene, and the resultant is washed with 300 ml of 1 N HCl and 500 ml of water $\times 3$  in this order. The monochlorobenzene solution is distilled off under reduced pressure to 30 ml, and the solution is added dropwise to 800 ml of ethyl acetate/methanol=1/3, to reprecipitate a polymer. The polymer thus obtained is filtered, washed with methanol, and then dried in a vacuum for 16 hours at  $60^\circ\text{C}$ . Thus, 0.6 g of a polymer (polymer compound 10) is obtained.

The molecular weight of this polymer is measured by gel permeation chromatography (GPC) (manufactured by Tosoh Corp., HLC-8120GPC), and it is found that  $M_w=6.7\times 10^4$  (relative to styrene standards), and  $M_w/M_n=2.2$ . The degree of polymerization,  $p$ , determined from the molecular weight of the monomer is about 80.



37

Synthesis Example 3

## Synthesis of Monomer Compound 7

4-Methylacetanilide (21.0 g) methyl 4-iodophenylpropionate (64.4 g), potassium carbonate (38.3 g), copper sulfate pentahydrate (2.3 g), and tridecane (50 ml) are introduced into a 500-ml three-necked flask, and the mixture is heated and stirred for 15 hours at 230° C. under a nitrogen gas stream.

After completion of the reaction, potassium hydroxide (15.6 g) dissolved in ethylene glycol (300 ml) is added thereto, and the mixture is heated to reflux for 3.5 hours under a nitrogen gas stream. Subsequently, the reaction liquid is cooled to room temperature (25° C.), and the reaction liquid is poured into 1 L of distilled water and neutralized with hydrochloric acid. Thus, crystals are precipitated out. The crystals are filtered by suction filtration, washed with water, and then transferred into a 1-L flask. Toluene (500 ml) is added to these crystals, and the mixture is heated to reflux. Water is removed by azeotropically boiling the mixture, and then a methanol (300 ml) solution of concentrated sulfuric acid (1.5 ml) is added thereto. The mixture is heated to reflux for 5 hours under a nitrogen gas stream.

After the reaction, the reaction mixture is extracted with toluene, and the organic layer is washed with pure water. Subsequently, the organic layer is dried over anhydrous sodium sulfate, and then the solvent is distilled off under reduced pressure. The residue is recrystallized from hexane, and thus 34.1 g of DAA-2 is obtained.



38

with hydrochloric acid. Thus, crystals are precipitated out. The crystals are filtered by suction filtration, washed with water, and then transferred into a 1-L flask. Toluene (500 ml) is added to these crystals, and the mixture is heated to reflux. Water is removed by azeotropically boiling the mixture, and then a methanol (300 ml) solution of concentrated sulfuric acid (1.5 ml) is added thereto. The mixture is heated to reflux for 5 hours under a nitrogen gas stream.

The mixture is cooled to room temperature (25° C.), toluene is added thereto, and the mixture is filtered through Celite. The filtrate is washed with pure water, the organic layer is extracted, and the organic solvent is distilled off. A product thus obtained is separated by silica gel column chromatography (hexane 4:toluene 1), and thus, 9.3 g of TAA-2 is obtained.



Under a nitrogen atmosphere, tetrahydrofuran (300 ml) is added to tetra(triphenylphosphine)palladium (0.54 g) and TAA-2 (8.5 g) in a 500-ml flask, and the mixture is stirred for 10 minutes. Subsequently, a 2 M aqueous solution of sodium carbonate (24.5 ml) and the diboronic acid compound (2.00 g) are added thereto, and the mixture is refluxed and magnetically stirred for 7 hours.

After completion of the reaction, ethyl acetate (100 ml) and water (50 ml) are added, and the mixture is thoroughly shaken to separate an organic layer and an aqueous layer. The aqueous layer is extracted with ethyl acetate (100 ml), and the respective organic layers are washed with saturated brine (100 ml) and dried over sodium sulfate. This organic layer is separated by silica gel column chromatography (ethyl acetate/hexane=1/3), and thus 1.1 g of a monomer compound 7 is obtained.

39

40



Monomer compound 7

It is confirmed by a  $^1\text{H}$ -NMR spectroscopic analysis and an IR spectroscopic analysis that the compound thus obtained is monomer compound 7.

#### Synthesis Example 4

##### Synthesis of Polymer Compound 12

1.0 g of the monomer compound 7 thus obtained, 10 ml of ethylene glycol, and 0.02 g of tetrabutoxytitanium are introduced into a 50-ml three-necked pear-shaped flask, and in a nitrogen atmosphere, the mixture is heated and stirred for 5 hours at 200° C.

After it is confirmed by TLC that the raw material monomer compound 7 has reacted and disappeared, the reaction mixture is heated to 210° C. while ethylene glycol is distilled off by lowering the pressure to 50 Pa, and the reaction is continued for 6 hours.

35 Thereafter, the reaction mixture is cooled to room temperature (25° C.), and is dissolved in 50 ml of tetrahydrofuran. Insoluble substances are filtered through a 0.5- $\mu\text{m}$  polytetrafluoroethylene (PTFE) filter, and the filtrate is distilled off under reduced pressure. The residue is dissolved in 300 ml of monochlorobenzene, and the resultant is washed with 300 ml of 1 N HCl and 500 ml of water $\times 3$  in this order. The 40 monochlorobenzene solution is distilled off under reduced pressure to 30 ml, and the solution is added dropwise to 800 ml of ethyl acetate/methanol=1/3, to reprecipitate a polymer. The polymer thus obtained is filtered, washed with methanol, and then dried in a vacuum for 16 hours at 60° C. Thus, 0.7 g 45 of a polymer (polymer compound 12) is obtained.

The molecular weight of this polymer is measured by gel permeation chromatography (GPC) (manufactured by Tosoh Corp., HLC-8120GPC), and it is found that  $M_w=5.8\times 10^4$  (relative to styrene standards), and  $M_w/M_n=2.3$ . The degree of polymerization,  $p$ , determined from the molecular weight of the monomer is about 67.



41

42

-continued



Polymer compound 12

## Synthesis Example 5

## Synthesis of Monomer Compound 17

1-Acetamidonaphthalene (25.0 g), methyl 4-iodophenylpropionate (64.4 g), potassium carbonate (38.3 g), copper sulfate pentahydrate (2.3 g), and tridecane (50 ml) are introduced into a 500-ml three-necked flask, and the mixture is heated and stirred for 18 hours at 230° C. under a nitrogen gas stream.

After completion of the reaction, potassium hydroxide (15.6 g) dissolved in ethylene glycol (300 ml) is added to the reaction liquid, and the mixture is heated to reflux for 3.5 hours under a nitrogen gas stream. Subsequently, the reaction liquid is cooled to room temperature (25° C.), and the reaction liquid is poured into 1 L of distilled water and is neutralized with hydrochloric acid. Thus, crystals are precipitated out. The crystals are filtered by suction filtration, and are washed with water, and then are transferred into a 1-L flask. Toluene (500 ml) is added to these crystals, and the mixture is heated to reflux. Water is removed by azeotropically boiling the mixture, and then a methanol (300 ml) solution of concentrated sulfuric acid (1.5 ml) is added thereto. The resulting mixture is heated to reflux for 5 hours under a nitrogen gas stream.

After the reaction, the mixture is extracted with toluene, and the organic layer is washed with pure water. Subsequently, the organic layer is dried over anhydrous sodium sulfate, subsequently the solvent is distilled off under reduced pressure, and the product is recrystallized from hexane. Thereby, 36.5 g of DAA-3 is obtained.



25

30

40

45

50

55

60

65

-continued



DAA-3

Subsequently, a mixed liquid of 1-bromo-4-iodobenzene (21.2 g), DAA-3 (20 g), copper(II) sulfate pentahydrate (1.0 g), potassium carbonate (5.0 g), and tridecane (12 ml) is stirred for 14 hours at 210° C.

After completion of the reaction, potassium hydroxide (15.6 g) dissolved in ethylene glycol (300 ml) is added to the reaction liquid, and the mixture is heated to reflux for 3.5 hours under a nitrogen gas stream. Subsequently, the reaction liquid is cooled to room temperature (25° C.), and the reaction liquid is poured into 1 L of distilled water and is neutralized with hydrochloric acid. Thus, crystals are precipitated out. The crystals are filtered by suction filtration, and are washed with water, and then are transferred into a 1-L flask. Toluene (500 ml) is added to these crystals, and the mixture is heated to reflux. Water is removed by azeotropically boiling the mixture, and then a methanol (300 ml) solution of concentrated sulfuric acid (1.5 ml) is added thereto. The resulting mixture is heated to reflux for 5 hours under a nitrogen gas stream.

The mixture is cooled to room temperature (25° C.), toluene is added thereto, and the mixture is filtered through Celite. The filtrate is washed with pure water, the organic layer is extracted, and the organic solvent is distilled off. A product thus obtained is separated by silica gel column chromatography (hexane 4:toluene 1), and thus, 14.5 g of TAA-3 is obtained.

**43**

-continued

**44**

After completion of the reaction, ethyl acetate (100 ml) and water (50 ml) are added thereto, and the mixture is thoroughly shaken to separate an organic layer and an aqueous layer. The aqueous layer is extracted with ethyl acetate (100 ml), and the respective organic layers are washed with saturated brine (100 ml) and dried over sodium sulfate. This organic layer is separated by silica gel column chromatography (ethyl acetate/hexane=1/3), and thus 1.4 g of a monomer compound 17 is obtained.



-continued

It is confirmed by a <sup>1</sup>H-NMR spectroscopic analysis and an IR spectroscopic analysis that the compound thus obtained is monomer compound 17.

45

Synthesis Example 6



In a nitrogen atmosphere, tetrahydrofuran (300 ml) is added to tetra(triphenylphosphine)palladium (0.537 g) and TAA-3 (8.8 g) in a 500-ml flask, and the mixture is stirred for 8 minutes. Subsequently, a 2 M aqueous solution of sodium carbonate (24.5 ml) and the diboronic acid compound II (2.00 g) are added, and the mixture is refluxed and magnetically stirred for 7 hours.

50

1.0 g of the monomer compound 17 thus obtained, 10 ml of ethylene glycol, and 0.02 g of tetrabutoxytitanium are introduced into a 50-ml three-necked pear-shaped flask, and in a nitrogen atmosphere, the mixture is heated and stirred for 5 hours at 200°C.

55

After it is confirmed by TLC that the raw material monomer compound 17 has reacted and disappeared, the reaction mixture is heated to 210°C. while ethylene glycol is distilled off by lowering the pressure to 50 Pa, and the reaction is continued for 6 hours.

60

Thereafter, the reaction mixture is cooled to room temperature (25°C.), and is dissolved in 50 ml of tetrahydrofuran. Insoluble substances are filtered through a 0.5-μm polytetrafluoroethylene (PTFE) filter, and the filtrate is distilled off under reduced pressure. Subsequently, the residue is dissolved in 300 ml of monochlorobenzene, and the resultant is washed with 300 ml of 1 N HCl and 500 ml of water<sup>3</sup> in this order. The monochlorobenzene solution is distilled off under

65

45

reduced pressure to 30 ml, and the solution is added dropwise to 800 ml of ethyl acetate/methanol=1/3, to reprecipitate a polymer. The polymer thus obtained is filtered, washed with methanol, and then dried in a vacuum for 16 hours at 60° C. Thus, 0.6 g of a polymer (polymer compound 20) is obtained.

The molecular weight of this polymer is measured by gel permeation chromatography (GPC) (manufactured by Tosoh Corp., HLC-8120GPC), and it is found that  $M_w=5.3\times 10^4$  (relative to styrene standards), and  $M_w/M_n=2.4$ . The degree of polymerization,  $p$ , determined from the molecular weight of the monomer is about 57.

46

Water is removed by azeotropically boiling the mixture, and then a methanol (300 ml) solution of concentrated sulfuric acid (1.5 ml) is added thereto. The mixture is heated to reflux for 5 hours under a nitrogen gas stream.

After the reaction, the reaction mixture is extracted with toluene, and the organic layer is washed with pure water. Subsequently, the organic layer is dried over anhydrous sodium sulfate, and then the solvent is distilled off under reduced pressure. The residue is recrystallized from hexane, and thus 17.9 g of DAA-4 is obtained.



Polymer compound 20

## Synthesis Example 7

## Synthesis of Monomer Compound 19

4-(2-thienyl)acetanilide (30.0 g), methyl 4-iodophenylpropiate (28.5 g), potassium carbonate (13.6 g), copper sulfate pentahydrate (2.0 g), and 1,2-dichlorobenzene (50 ml) are introduced into a 500-ml three-necked flask, and the mixture is heated and stirred for 12 hours at 230° C. under a nitrogen gas stream.

After completion of the reaction, potassium hydroxide (15.6 g) dissolved in ethylene glycol (300 ml) is added thereto, and the mixture is heated to reflux for 3.5 hours under a nitrogen gas stream. Subsequently, the reaction liquid is cooled to room temperature (25° C.), and the reaction liquid is poured into 1 L of distilled water and neutralized with hydrochloric acid. Thus, crystals are precipitated out. The crystals are filtered by suction filtration, washed with water, and then transferred into a 1-L flask. Toluene (500 ml) is added to these crystals, and the mixture is heated to reflux.



In a nitrogen atmosphere, a liquid mixture of 1-bromo-4-iodobenzene (15.9 g), DAA-4 (16.0 g), copper(II) sulfate pentahydrate (0.2 g), potassium carbonate (1.3 g), and tridecane (15 ml) is stirred for 15 hours at 210° C.

After completion of the reaction, potassium hydroxide (15.6 g) dissolved in ethylene glycol (300 ml) is added thereto, and the mixture is heated to reflux for 3.5 hours under

47

a nitrogen gas stream. Subsequently, the reaction liquid is cooled to room temperature (25° C.), and the reaction liquid is poured into 1 L of distilled water and neutralized with hydrochloric acid. Thus, crystals are precipitated out. The crystals are filtered by suction filtration, washed with water, and then transferred into a 1-L flask. Toluene (500 ml) is added to these crystals, and the mixture is heated to reflux. Water is removed by azeotropically boiling the mixture, and then a methanol (300 ml) solution of concentrated sulfuric acid (1.5 ml) is added thereto. The mixture is heated to reflux for 5 hours under a nitrogen gas stream. 5

After the mixture is cooled, toluene is added thereto, and the mixture is filtered through Celite. Toluene is distilled off, and a product thus obtained is separated by silica gel column chromatography (hexane 2:toluene 1), and thus 9.1 g of TAA-4 is obtained. 10 15



48



Under a nitrogen atmosphere, tetrahydrofuran (250 ml) is added to tetra(triphenylphosphine)palladium (0.54 g) and TAA-4 (8.6 g) in a 500-ml flask, and the mixture is stirred for 10 minutes. Subsequently, a 2 M aqueous solution of sodium carbonate (24.5 ml) and the diboronic acid compound (2.00 g) are added thereto, and the mixture is refluxed and magnetically stirred for 7 hours. 20

After completion of the reaction, ethyl acetate (100 ml) and water (50 ml) are added, and the mixture is thoroughly shaken to separate an organic layer and an aqueous layer. The aqueous layer is extracted with ethyl acetate (100 ml), and the respective organic layers are washed with saturated brine (100 ml) and dried over sodium sulfate. This organic layer is 25 separated by silica gel column chromatography (ethyl acetate/hexane=1/3), and thus 1.2 g of a monomer compound 19 is obtained. 30



**49**

It is confirmed by a  $^1\text{H-NMR}$  spectroscopic analysis and an IR spectroscopic analysis that the compound thus obtained is monomer compound 19.

## Synthesis Example 8

## Synthesis of Polymer Compound 22

1.0 g of the monomer compound 19 thus obtained, 10 ml of ethylene glycol and 0.02 g of tetrabutoxytitanium are intro-

**50**

ml of ethyl acetate/methanol=1/3, to reprecipitate a polymer. The polymer thus obtained is filtered, washed with methanol, and then dried in a vacuum for 16 hours at 60° C. Thus, 0.6 g of a polymer (polymer compound 22) is obtained.

The molecular weight of this polymer is measured by gel permeation chromatography (GPC) (manufactured by Tosoh Corp., HLC-8120GPC), and it is found that  $M_w=6.8\times 10^4$  (relative to styrene standards), and  $M_w/M_n=2.1$ . The degree of polymerization,  $p$ , determined from the molecular weight of the monomer is about 68.



Polymer compound 22

duced into a 50-ml three-necked pear-shaped flask, and in a nitrogen atmosphere, the mixture is heated and stirred for 5 hours at 200° C.

After it is confirmed by TLC that the raw material monomer compound 19 has reacted and disappeared, the reaction mixture is heated to 210° C. while ethylene glycol is distilled off by lowering the pressure to 50 Pa, and the reaction is continued for 6 hours.

Thereafter, the reaction mixture is cooled to room temperature (25° C.), and is dissolved in 50 ml of tetrahydrofuran. Insoluble substances are filtered through a 0.5-μm polytetrafluoroethylene (PTFE) filter, and the filtrate is distilled off under reduced pressure. The residue is dissolved in 300 ml of monochlorobenzene, and the resultant is washed with 300 ml of 1 N HCl and 500 ml of water $\times 3$  in this order. The monochlorobenzene solution is distilled off under reduced pressure to 30 ml, and the solution is added dropwise to 800

50

## Synthesis Example 9

## Synthesis of Monomer Compound 23

Under a nitrogen atmosphere, 2-iodo-9,9-dimethylfluorene (31.8 g), methyl 4-acetaminophenylpropionate (20.0 g), potassium carbonate (18.8 g), copper sulfate pentahydrate (1.2 g), and tridecane (15 ml) are introduced into a 300-ml three-necked flask, and the mixture is heated and stirred for 13 hours at 200° C. under a nitrogen gas stream.

After completion of the reaction, 150 ml of ethylene glycol and 7.6 g of potassium hydroxide are added thereto, and the mixture is heated to reflux for 5 hours under a nitrogen gas stream. Subsequently, the mixture is cooled to room temperature (25° C.), and this is poured into 150 ml of distilled water and neutralized with hydrochloric acid. Thus, crystals are precipitated out. These crystals are filtered, washed with

55

60

65

51

water, and then transferred into a 500-ml flask. 500 ml of toluene is added to these crystals, and the mixture is heated to reflux. Water is removed by azeotropically boiling the mixture, and then 100 ml of methanol and 1.0 ml of concentrated sulfuric acid are added thereto. The mixture is heated to reflux for 5 hours under a nitrogen gas stream.

After the reaction, the reaction mixture is extracted with toluene, and the organic layer is washed with distilled water. Subsequently, the organic layer is dried over anhydrous sodium sulfate, and then the solvent is distilled off under reduced pressure. The residue is recrystallized from hexane, and thus 25 g of DAA-5 is obtained.



Subsequently, a liquid mixture of 1-bromo-4-iodobenzene (21.2 g), DAA-5 (20 g), copper(II) sulfate pentahydrate (1.0 g), potassium carbonate (4.5 g), and tridecane (10 ml) is stirred for 8 hours at 210°C.

After completion of the reaction, 150 ml of ethylene glycol and 7.6 g of potassium hydroxide are added thereto, and the mixture is heated to reflux for 5 hours under a nitrogen gas stream. Subsequently, the reaction mixture is cooled to room temperature (25°C), and this is poured into 150 ml of distilled water and neutralized with hydrochloric acid. Thus, crystals are precipitated out. These crystals are filtered, washed with water, and then transferred into a 500-ml flask. 500 ml of toluene is added to these crystals, and the mixture is heated to reflux. Water is removed by azeotropically boiling the mixture, and then 100 ml of methanol and 1.0 ml of concentrated sulfuric acid are added thereto. The mixture is heated to reflux for 5 hours under a nitrogen gas stream.

The mixture is cooled to room temperature (25°C), toluene is added thereto, and the mixture is filtered through Celite. 60 The filtrate is washed with pure water, the organic layer is extracted, and the organic solvent is distilled off. A product

52

thus obtained is separated by silica gel column chromatography (hexane 4:toluene 1), and thus 15.6 g of TAA-5 is obtained.



Under a nitrogen atmosphere, tetrahydrofuran (250 ml) is added to tetra(triphenylphosphine)palladium (0.54 g) and TAA-5 (8.8 g) in a 500-ml flask, and the mixture is stirred for 10 minutes. Subsequently, a 2 M aqueous solution of sodium carbonate (24.5 ml) and the diboronic acid compound (2.00 g) are added thereto, and the mixture is refluxed and magnetically stirred for 7 hours.

After completion of the reaction, ethyl acetate (100 ml) and water (50 ml) are added, and the mixture is thoroughly shaken to separate an organic layer and an aqueous layer. The aqueous layer is extracted with ethyl acetate (100 ml), and the respective organic layers are washed with saturated brine (100 ml) and dried over sodium sulfate. This organic layer is separated by silica gel column chromatography (ethyl acetate/hexane=1/3), and thus 1.2 g of a monomer compound 65 23 is obtained.



### Monomer compound 23

It is confirmed by a  $^1\text{H}$ -NMR spectroscopic analysis and an IR spectroscopic analysis that the compound thus obtained is monomer compound 23.

### Synthesis Example 10

## Synthesis of Polymer Compound 23

1.0 g of the monomer compound 23 thus obtained, 10 ml of ethylene glycol, and 0.02 g of tetrabutoxytitanium are introduced into a 50-ml three-necked pear-shaped flask, and the mixture is heated and stirred for 5 hours at 200° C. in a nitrogen atmosphere.

After it is confirmed by TLC that the raw material monomer compound 23 has reacted and disappeared, the reaction mixture is heated to 210° C. while ethylene glycol is distilled off by lowering the pressure to 50 Pa, and the reaction is continued for 6 hours.

Thereafter, the reaction mixture is cooled to room temperature (25° C.), and is dissolved in 50 ml of tetrahydrofuran. Insoluble substances are filtered through a 0.5-µm polytetrafluoroethylene (PTFE) filter, and the filtrate is distilled off under reduced pressure. The residue is dissolved in 300 ml of monochlorobenzene, and the resultant is washed with 300 ml of 1 N HCl and 500 ml of water×3 in this order. The monochlorobenzene solution is distilled off under reduced pressure to 30 ml, and the solution is added dropwise to 800 ml of ethyl acetate/methanol=1/3, to reprecipitate a polymer. The polymer thus obtained is filtered, washed with methanol, and then dried in a vacuum for 16 hours at 60° C. Thus, 0.6 g of a polymer (polymer compound 23) is obtained.

The molecular weight of this polymer is measured by gel permeation chromatography (GPC) (manufactured by Tosoh Corp., HLC-8120GPC), and it is found that  $M_w=8.9\times 10^4$  (relative to styrene standards), and  $M_w/M_n=2.4$ . The degree of polymerization,  $p$ , determined from the molecular weight of the monomer is about 83.



Polymer compound 23

## Synthesis Example 11

## Synthesis of Monomer Compound 15

Under a nitrogen atmosphere, 23 g of 3-bromobiphenyl, 20 g of methyl 4-acetaminophenylpropionate, 18.8 g of potassium carbonate, 1.1 g of copper sulfate pentahydrate, and 20 ml of tridecane are introduced into a 300-ml three-necked flask, and the mixture is heated and stirred for 24 hours at 200° C. under a nitrogen gas stream.

After completion of the reaction, 150 ml of ethylene glycol and 6.5 g of potassium hydroxide are added thereto, and the mixture is heated to reflux for 3 hours under a nitrogen gas stream. Subsequently, the reaction mixture is cooled to room temperature (25° C.), and this is poured into 150 ml of distilled water and neutralized with hydrochloric acid. Thus, crystals are precipitated out. These crystals are filtered, washed with water, and then transferred into a 500-ml flask. 500 ml of toluene is added to these crystals, and the mixture is heated to reflux. Water is removed by azeotropically boiling the mixture, and then 100 ml of methanol and 1.0 ml of concentrated sulfuric acid are added thereto. The mixture is heated to reflux for 5 hours under a nitrogen gas stream.

After the reaction, the reaction mixture is extracted with toluene, and the organic layer is washed with distilled water. Subsequently, the organic layer is dried over anhydrous sodium sulfate, and then the solvent is distilled off under

reduced pressure. The residue is recrystallized from hexane, and thus 25 g of DAA-6 is obtained.



57

Subsequently, a liquid mixture of 1-bromo-4-iodobenzene (15.9 g), DAA-6 (15 g), copper(II) sulfate pentahydrate (0.6 g), potassium carbonate (3.9 g), and tridecane (10 ml) is stirred for 10 hours at 210° C.

After completion of the reaction, 150 ml of ethylene glycol and 6.5 g of potassium hydroxide are added thereto, and the mixture is heated to reflux for 3 hours under a nitrogen gas stream. Subsequently, the reaction mixture is cooled to room temperature (25° C.), and this is poured into 150 ml of distilled water and neutralized with hydrochloric acid. Thus, 5 crystals are precipitated out. These crystals are filtered, washed with water, and then transferred into a 500-ml flask. 10 500 ml of toluene is added to these crystals, and the mixture is heated to reflux. Water is removed by azeotropically boiling the mixture, and then 100 ml of methanol and 1.0 ml of concentrated sulfuric acid are added thereto. The mixture is 15 heated to reflux for 5 hours under a nitrogen gas stream.

The reaction mixture is cooled to room temperature (25° C.), toluene is added thereto, and the mixture is filtered through Celite. The filtrate is washed with pure water, and the organic layer is extracted. The organic solvent is distilled off, and a product thus obtained is separated by silica gel column chromatography (hexane 4:toluene 1). Thus, 11.7 g of TAA-6 20 is obtained.



58

-continued



Under a nitrogen atmosphere, tetrahydrofuran (250 ml) is added to tetra(triphenylphosphine)palladium (0.54 g) and TAA-6 (8.6 g) in a 500-ml flask, and the mixture is stirred for 10 minutes. Subsequently, a 2 M aqueous solution of sodium 25 carbonate (24.5 ml) and the diboronic acid compound (2.00 g) are added thereto, and the mixture is refluxed and magnetically stirred for 7 hours.

After completion of the reaction, ethyl acetate (100 ml) and 30 water (50 ml) are added, and the mixture is thoroughly shaken to separate an organic layer and an aqueous layer. The aqueous layer is extracted with ethyl acetate (100 ml), and the respective organic layers are washed with saturated brine 35 (100 ml) and dried over sodium sulfate. This organic layer is separated by silica gel column chromatography (ethyl acetate/hexane=1/3), and thus 1.2 g of a monomer compound 15 is obtained.



Monomer compound 15

59

It is confirmed by a  $^1\text{H-NMR}$  spectroscopic analysis and an IR spectroscopic analysis that the compound thus obtained is monomer compound 15.

### Synthesis Example 12

## Synthesis of Polymer Compound 18

1.0 g of the monomer compound 15 thus obtained, 10 ml of ethylene glycol and 0.02 g of tetrabutoxytitanium are intro-

60

(relative to styrene standards), and  $M_w/M_n=2.2$ . The degree of polymerization,  $p$ , determined from the molecular weight of the monomer is about 49.

5

### Synthesis Example 13

## Synthesis of Monomer Compound 31

Under a nitrogen atmosphere, 25.6 g of 9-bromophenanthrene, 20.0 g of methyl 4-acetaminophenylpropionate, 18.8



### Polymer compound 18

duced into a 50-ml three-necked pear-shaped flask, and under a nitrogen atmosphere, the mixture is heated and stirred for 5 hours at 200° C.

After it is confirmed by TLC that the raw material monomer compound 15 has reacted and disappeared, the reaction mixture is heated to 210° C. while ethylene glycol is distilled off by lowering the pressure to 50 Pa, and the reaction is continued for 6 hours.

Thereafter, the reaction mixture is cooled to room temperature ( $25^{\circ}\text{ C.}$ ), and is dissolved in 50 ml of tetrahydrofuran. Insoluble substances are filtered through a  $0.5\text{-}\mu\text{m}$  polytetrafluoroethylene (PTFE) filter, and the filtrate is distilled off under reduced pressure. The residue is dissolved in 300 ml of monochlorobenzene, and the resultant is washed with 300 ml of 1 N HCl and 500 ml of water $\times 3$  in this order. The monochlorobenzene solution is distilled off under reduced pressure to 30 ml, and the solution is added dropwise to 800 ml of ethyl acetate/methanol=1/3, to reprecipitate a polymer. The polymer thus obtained is filtered, washed with methanol, and then dried in a vacuum for 16 hours at  $60^{\circ}\text{ C.}$  Thus, 0.6 g of a polymer (polymer compound 18) is obtained.

The molecular weight of this polymer is measured by gel permeation chromatography (GPC) (manufactured by Tosoh Corp., HLC-8120GPC), and it is found that  $M_w = 4.9 \times 10^4$

45 g of potassium carbonate, 1.2 g of copper sulfate pentahydrate, and 15 ml of tridecane are introduced into a 300-ml three-necked flask, and the mixture is heated and stirred for 13 hours at 200° C. under a nitrogen gas stream.

After completion of the reaction, 150 ml of ethylene glycol and 7.6 g of potassium hydroxide are added thereto, and the reaction mixture is heated to reflux for 5 hours under a nitrogen gas stream. Subsequently, the reaction mixture is cooled to room temperature (25° C.), and this is poured into 150 ml of distilled water and neutralized with hydrochloric acid. Thus, crystals are precipitated out. These crystals are filtered, sufficiently washed with water, and then transferred into a 500-ml flask. 500 ml of toluene is added to these crystals, and the mixture is heated to reflux. Water is removed by azeotropically boiling the mixture, and then 100 ml of methanol and 1.0 ml of concentrated sulfuric acid are added thereto. The mixture is heated to reflux for 5 hours under a nitrogen gas stream.

After the reaction, the reaction mixture is extracted with toluene, and the organic layer is washed sufficiently with distilled water. Subsequently, the organic layer is dried over anhydrous sodium sulfate, and then the solvent is distilled off under reduced pressure. The residue is recrystallized from hexane, and thus 25 g of DAA-7 is obtained.

61



62



Subsequently, a liquid mixture of 1-bromo-4-iodobenzene (21.2 g), DAA-7 (19.1 g), copper(II) sulfate pentahydrate (1.0 g), potassium carbonate (4.5 g), and tridecane (10 ml) is stirred for 8 hours at 210° C.

After completion of the reaction, 150 ml of ethylene glycol and 6.5 g of potassium hydroxide are added thereto, and the reaction mixture is heated to reflux for 3 hours under a nitrogen gas stream. Subsequently, the reaction mixture is cooled to room temperature (25° C.), and this is poured into 150 ml of distilled water and neutralized with hydrochloric acid. Thus, crystals are precipitated out. These crystals are filtered, washed with water, and then transferred into a 500-ml flask. 500 ml of toluene is added to these crystals, and the mixture is heated to reflux. Water is removed by azeotropically boiling the mixture, and then 100 ml of methanol and 1.0 ml of concentrated sulfuric acid are added thereto. The mixture is heated to reflux for 5 hours under a nitrogen gas stream.

The reaction mixture is cooled to room temperature (25° C.), toluene is added thereto, and the mixture is filtered through Celite. The filtrate is washed with pure water, and the organic layer is extracted. The organic solvent is distilled off, and a product thus obtained is separated by silica gel column chromatography (hexane 4:toluene 1). Thus, 15.6 g of TAA-7 is obtained.

In a nitrogen atmosphere, tetrahydrofuran (250 ml) is added to tetra(triphenylphosphine)palladium (0.54 g) and TAA-7 (8.5 g) in a 500-ml flask, and the mixture is stirred for 10 minutes. Subsequently, a 2 M aqueous solution of sodium carbonate (24.5 ml) and the diboronic acid compound (2.00 g) are added, and the mixture is refluxed and magnetically stirred for 7 hours.

After completion of the reaction, ethyl acetate (100 ml) and water (50 ml) are added thereto, and the mixture is thoroughly shaken to separate an organic layer and an aqueous layer. The aqueous layer is extracted with ethyl acetate (100 ml), and the respective organic layers are washed with saturated brine (100 ml) and dried over sodium sulfate. This organic layer is separated by silica gel column chromatography (ethyl acetate/hexane=1/3), and thus 1.0 g of a monomer compound 31 is obtained.



63

64

-continued



Monomer compound 31

It is confirmed by a  $^1\text{H}$ -NMR spectroscopic analysis and an IR spectroscopic analysis that the compound thus obtained is monomer compound 31.

Production of Image Holding Member for Image Forming Apparatus

Example 1

A solution formed from 10 parts by weight of a zirconium compound (ORGATIX ZC540, manufactured by Matsumoto Seiyaku K.K.), 1 part by weight of a silane compound (A1110, manufactured by Nippon Unicar Co., Ltd.), 40 parts by weight of i-propanol, and 20 parts by weight of butanol is applied on an aluminum substrate by a dip coating method, and the solution is heated to dry for 10 minutes at 150°C. Thus, an undercoat layer having a thickness of 0.6  $\mu\text{m}$  is formed. One part by weight of chlorogallium phthalocyanine crystals having strong peaks at Bragg angles ( $20\pm0.2^\circ$ ) of 7.4°, 16.6°, 25.5° and 28.3° in the X-ray diffraction spectrum, is mixed with 1 part by weight of a polyvinyl butyral resin (S-LEC BM-S, manufactured by Sekisui Chemical Co., Ltd.) and 100 parts by weight of n-butyl acetate, and the mixture is dispersed by treating the mixture with a paint shaker together with glass beads for one hour. Subsequently, a coating liquid thus obtained is applied on the undercoat layer by a dip coating method, and is heated to dry for 10 minutes at 100°C. Thus, a charge generating layer is formed.

Subsequently, 2 parts by weight of the monomer compound 6 obtained as described above and 3 parts by weight of a bisphenol (Z) polymer compound having the structure shown below (viscosity average molecular weight: 40,000) are heated and dissolved in 35 parts by weight of chlorobenzene, and then the solution is returned to room temperature (25°C.). This coating liquid is applied on the charge generating layer by a dip coating method, and is heated for 60 minutes at 130°C. Thus, a charge transport layer having a thickness of 20  $\mu\text{m}$  is formed.



Bisphenol (Z) polymer compound

Example 2 to Example 13

Image holding members for image forming apparatuses are produced in the same manner as in Example 1, except that the polymer compound 10, the monomer compound 7, the polymer compound 12, the monomer compound 17, the polymer compound 20, the monomer compound 19, the polymer compound 22, the monomer compound 23, the polymer compound 23, the monomer compound 15, the polymer compound 18 and the monomer compound 31 are respectively used instead of the monomer compound 6 used in Example 1.

Example 14

An image holding member for an image forming apparatus is produced in the same manner as in Example 1, except that hydroxygallium phthalocyanine crystals having strong diffraction peaks at Bragg angles ( $20\pm0.2^\circ$ ) of 7.5°, 9.9°, 12.5°, 16.3°, 18.6°, 25.1° and 28.3° in the X-ray diffraction spectrum are used instead of the chlorogallium phthalocyanine crystals used in Example 1.

Comparative Example 1

An image holding member for an image forming apparatus is produced by the method described in Example 1, except that a compound (X) having the following structure is used instead of Specific Example compound 6 used in Example 1.



## Comparative Example 2

An image holding member for an image forming apparatus is produced by the method described in Example 1, except that a compound (XI) having the following structure (p=52) is used instead of Specific Example compound 6 used in Example 1.

(XI)



## Comparative Example 3

An image holding member for an image forming apparatus is produced by the method described in Example 1, except that a compound (XII) having the following structure is used instead of Specific Example compound 6 used in Example 1.

(XII)



## Comparative Example 4

An image holding member for an image forming apparatus is produced by the method described in Example 1, except that a compound (XIII) having the following structure (p=55) is used instead of Specific Example compound 6 used in Example 1.



## Evaluation

In order to evaluate electrophotographic characteristics using the respective image holding members for image forming apparatuses obtained in the Examples and Comparative Examples described above, each of the image holding members is charged by performing corona discharge at -6 kV in an environment at 20° C. and 40% RH using an electrostatic duplicating paper testing device (ELECTROSTATIC ANALYZER EPA-8100, manufactured by Kawaguchi Electric Works Co., Ltd.), and then the light of a tungsten lamp is converted to monochromatic light at 800 nm using a monochromator and is irradiated in an amount adjusted to be 1  $\mu\text{W}/\text{cm}^2$  on the surface of the photoreceptor.

Then, the surface potential  $V_0$  (V) of the photoreceptor surface immediately after charging, and the half decay exposure  $E1/2$  ( $\text{erg}/\text{cm}^2$ ) at which the surface potential becomes  $1/2 \times V_0$  (V) as a result of light irradiation of the photoreceptor surface, are measured (initial characteristics). Thereafter, white light at 10 lux is irradiated for one second, and the residual potential VRP (V) remaining on the photoreceptor surface is measured (initial characteristics).

Furthermore, the values of  $V_0$ ,  $E1/2$  and VRP are measured after repeating 1000 times the processes of charging, exposure (monochromatic light at 800 nm, the amount of exposure is the half decay exposure), and irradiation with white light (10 lux). Furthermore, the amounts of variance,  $\Delta V_0$ ,  $\Delta E1/2$ , and  $\Delta \text{VRP}$  are evaluated (stability and durability).

Next, image forming apparatuses are produced using the image holding members for image forming apparatuses obtained in the Examples and Comparative Examples. As elements other than the image holding member for an image forming apparatus, those mounted in a printer manufactured by Fuji Xerox Co., Ltd., DOCUCENTER C6550I, are used.

(XIII)

25

For each of the image forming apparatuses, an image forming test is carried out on 10,000 sheets (image density 10%, cyan 100%) in an environment of 28° C. and 75% RH. Meanwhile, under these test conditions, the process of each cartridge is carried out routinely, but toners of the cartridge other than the cyan toner are not used (supplied). After the test, the toner cleaning properties (staining of the charger due to poor cleaning, or deterioration of image quality), and the image quality (fine line reproducibility at 1 dot process black and a line slope of 45°) are evaluated. The methods for evaluation and the evaluation criteria for the cleaning properties and the image quality are as follows, and the obtained results are presented in Table 1.

The cleaning properties are evaluated by visual inspection, and are evaluated based on the following evaluation criteria.

A: Good

B: Partially having streaky image defects (about 10% or less of the entirety)

C: Having streaky image defects over a wide area

The image quality is examined using a magnifying glass, and is evaluated based on the following evaluation criteria.

A: Good

B: Partially having defects (no problem for practical use)

C: Having defects (fine lines are not reproduced)

TABLE 1

| Example   | Initial characteristics<br>(first time) |                                        |            | Maintenance<br>characteristics |                                        |            | Stability | Durability                                    |                     |                            |                        |
|-----------|-----------------------------------------|----------------------------------------|------------|--------------------------------|----------------------------------------|------------|-----------|-----------------------------------------------|---------------------|----------------------------|------------------------|
|           | $V_0$<br>(V)                            | $E1/2$<br>( $\text{erg}/\text{cm}^2$ ) | VRP<br>(V) | $V_0$<br>(V)                   | $E1/2$<br>( $\text{erg}/\text{cm}^2$ ) | VRP<br>(V) |           | $\Delta E1/2$<br>( $\text{erg}/\text{cm}^2$ ) | $\Delta V_0$<br>(V) | $\Delta \text{VRP}$<br>(V) | Cleaning<br>properties |
| Example 1 | -801                                    | 2.4                                    | -12        | -790                           | 2.8                                    | -22        | 0.3       | 11                                            | 10                  | A                          | A                      |
| Example 2 | -800                                    | 2.4                                    | -12        | -791                           | 2.8                                    | -24        | 0.4       | 10                                            | 12                  | A                          | A                      |
| Example 3 | -799                                    | 2.4                                    | -11        | -788                           | 2.8                                    | -22        | 0.4       | 11                                            | 11                  | A                          | B                      |
| Example 4 | -805                                    | 2.5                                    | -10        | -795                           | 2.8                                    | -20        | 0.3       | 10                                            | 10                  | A                          | A                      |
| Example 5 | -803                                    | 2.5                                    | -14        | -793                           | 2.7                                    | -23        | 0.3       | 10                                            | 9                   | A                          | B                      |
| Example 6 | -796                                    | 2.5                                    | -11        | -782                           | 2.9                                    | -22        | 0.4       | 14                                            | 11                  | A                          | A                      |
| Example 7 | -802                                    | 2.4                                    | -10        | -790                           | 2.8                                    | -20        | 0.4       | 10                                            | 12                  | A                          | A                      |

TABLE 1-continued

From the results described above, it can be seen that the image holding members for image forming apparatuses obtained in the Examples of the present invention have small variances in the residual potential due to repeated use, as compared with the Comparative Examples. Furthermore, it can be seen that the images obtained by the image forming apparatuses having the image holding members for image forming apparatuses have satisfactory image quality.

The foregoing description of the exemplary embodiments of the present invention has been provided for the purposes of illustration and description. It is not intended to be exhaustive or to limit the invention to the precise forms disclosed. Obviously, many modifications and variations will be apparent to practitioners skilled in the art. The embodiments were chosen and described in order to best explain the principles of the invention and its practical applications, thereby enabling others skilled in the art to understand the invention for various embodiments and with the various modifications as are suited to the particular use contemplated. It is intended that the scope of the invention be defined by the following claims and their equivalents.

What is claimed is:

1. An image holding member for an image forming apparatus, comprising a support, and a photosensitive layer disposed on the support and containing a compound represented by the following formula (I):



wherein in the formula (I), R<sup>1</sup>'s each independently represent a substituted or unsubstituted, linear or branched alkyl group having from 1 to 8 carbon atoms; Ar's each independently represent a substituted or unsubstituted phenyl group, a substituted or unsubstituted monovalent polynuclear aromatic hydrocarbon group having two aromatic rings, a substituted or unsubstituted monovalent condensed aromatic hydrocarbon group having two or three aromatic rings, or a substituted or unsubstituted monovalent aromatic heterocyclic group; and n's each independently represent a number of from 0 to 7.

2. A process cartridge, comprising:  
the image holding member for an image forming apparatus  
according to claim 1; and  
at least one selected from a charging unit that charges the  
image holding member for an image forming apparatus,  
an exposure unit that exposes the charged image holding  
member for an image forming apparatus to form an  
electrostatic latent image, a developing unit that devel-  
ops the electrostatic latent image to form a toner image,  
a transfer unit that transfers the toner image to a transfer  
medium, and a cleaning unit that cleans the image hold-  
ing member for an image forming apparatus.

3. An image forming apparatus, comprising:  
the image holding member for an image forming apparatus  
according to claim 1;  
a charging unit that charges the image holding member for  
an image forming apparatus;  
an exposure unit that exposes the charged image holding  
member for an image forming apparatus to form an  
electrostatic latent image;  
a developing unit that develops the electrostatic latent  
image to form a toner image; and

71

a transfer unit that transfers the toner image to a transfer medium.

4. An image holding member for an image forming apparatus, comprising a support, and a photosensitive layer disposed on the support and containing a compound represented by the following formula (II-1):

Formula (II-1) 10



15

wherein in the formula (II-1),  $Y^1$ 's each independently represent a substituted or unsubstituted divalent hydrocarbon group;  $A^1$  represents a group represented by the following formula (II-2);  $R^2$ 's each independently represent a hydrogen atom, an alkyl group, a substituted or unsubstituted aryl group, or a substituted or unsubstituted aralkyl group;  $m$ 's each independently represent an integer of from 1 to 5; and  $p$  represents an integer of from 5 to 5,000:

20

25

(II-2)



30

35

40

72

wherein in the formula (II-2),  $Ar$ 's each independently represent a substituted or unsubstituted phenyl group, a substituted or unsubstituted monovalent polynuclear aromatic hydrocarbon group having two aromatic rings, a substituted or unsubstituted monovalent condensed aromatic hydrocarbon group having two or three aromatic rings, or a substituted or unsubstituted monovalent aromatic heterocyclic group; and  $n$ 's each independently represent a number of from 0 to 7.

5. A process cartridge, comprising:

the image holding member for an image forming apparatus according to claim 4; and

at least one selected from a charging unit that charges the image holding member for an image forming apparatus, an exposure unit that exposes the charged image holding member for an image forming apparatus to form an electrostatic latent image, a developing unit that develops the electrostatic latent image to form a toner image, a transfer unit that transfers the toner image to a transfer medium, and a cleaning unit that cleans the image holding member for an image forming apparatus.

6. An image forming apparatus, comprising:

the image holding member for an image forming apparatus according to claim 4;

a charging unit that charges the image holding member for an image forming apparatus;

an exposure unit that exposes the charged image holding member for an image forming apparatus to form an electrostatic latent image;

a developing unit that develops the electrostatic latent image to form a toner image; and

a transfer unit that transfers the toner image to a transfer medium.

\* \* \* \* \*